# EUROPEAN PATENT SPECIFICATION

(11) **EP 1 908 878 B1**
(45) Date of publication and mention of the grant of the patent: **11.04.2012**
(21) Application number: 06757356.8
(22) Date of filing: 15.06.2006
(51) Int. Cl.: D21H 19/82, D21H 23/34, D21H 23/56, D21H 25/06, D21H 19/84

(54) **PROCESS FOR PRODUCING COATED PAPER AND COATED PAPER**
VERFAHREN ZUR HERSTELLUNG VON BESCHICHTETEM PAPIER UND BESCHICHTETES PAPIER
PROCÉDÉ DE FABRICATION DE PAPIER COUCHÉ ET PAPIER COUCHÉ

(30) Priority: 20.06.2005 JP 2005179111; 17.11.2005 JP 2005332733
(43) Date of publication of application: 09.04.2008
(73) Proprietor: DAIO PAPER CORPORATION, Shikokuchuo-shi, Ehime 799-0492 (JP)
(72) Inventor: MATSUSHIMA, Tadahiro, c/o DAIO PAPER CORPORATION, Shikokuchuo-shi, Ehime 799-0492 (JP)
(74) Representative: Held, Stephan
(86) International application number: PCT/JP2006/312058
(87) International publication number: WO 2006/137328

(56) References cited:
- EP-A2- 0 726 353
- WO-A1-03/052204
- JP-A- 09 291 490
- JP-A- 10 259 594
- JP-A- 11 001 891
- JP-A- 11 050 392
- JP-A- 11 279 992
- JP-A- 2000 303 382
- JP-A- 2005 146 444
- JP-A- 2006 138 045
- US-A- 5 118 533
- US-A- 5 169 715

## Description

### Technical Field

The present invention relates to a process and apparatus for producing a coated paper.
In particular, the present invention involves using, as means for forming coating layers on a surface of a base paper, coating apparatuses differing in coating method, for example, coating apparatuses including a combination of a roll coater and a blade coater that form at least two coating layers on a surface layer of the base paper. The present invention suitably relates to a process for producing a coated paper that can efficiently carry out production with high quality at a speed of 1300 m/min or more, particularly at a high speed of 1550 m/min or more integratedly from paper to finally finished products by means of on-machine technology, and coated paper.

### Background Art

In response to recent promotion of visualization and changes to multimedia, needs have been rapidly increased to highly qualify such as to visualize and colorize even printed matters having been widely used as media such as publications, advertisements, and posters. With changes in such user demands, an increase in the replacement of a conventional uncoated printing paper by a coated paper for printing rapidly leads to increasing demand for the coated paper for printing.

In addition, printing steps more and more severely request the qualities of handling properties of printing paper and traveling stability on a printer, which are involved in improvement in workability and efficiency.

Of the quality requests, paper manufacturing industries have implemented involvements with wider and more highly speedy paper machines in order to save energy and reduce manufacturing costs.

In the quality request for a coated paper and power saving and manufacturing cost reduction, the trend lies in lower grams per square meter of a base paper and ultra lightweight coating. In manufacturing premises, reformation is strongly invoked for techniques of producing a coated paper for printing having more excellent printing properties while maintaining characteristics of high-speed running ability.

In response to these quality demands, a technique is disclosed that involves, in an offset printing paper to be coated including an undercoat coated layer having a pigment and an adhesive and an overcoat coated layer, containing in a base paper 3 to 20 weight % of a needle or columnar soft calcium carbonate as an internal loading material based on the weight of the base paper, containing in the undercoat coated layer a styrene/butadiene copolymer latex having a gel content of from 75 to 90 weight % and having an average particle diameter of from 40 to 70 mm, and containing in the overcoat coated layer a styrene/butadiene copolymer latex having a gel content of from 40 to 70 weight % and having an average particle diameter of from 40 to 80 mm (Patent Document 1). Also disclosed is a process of producing a to-be-coated paper for applying a coating liquid having a pigment and an adhesive to a paper base, in which a wet paper is water-squeezed using a shoe press in a press part of a base paper machine, the dried base paper and/or undercoat coated paper produced by applying a coating liquid to the base paper is treated by means of a soft calender constituted by a metal roll and an elastic roll at a metal roll surface temperature of from 40 to 90°C at a linear pressure of from 30 to 150 kg/cm, and then a coating liquid having a pigment and an adhesive is applied thereto (Patent Document 2).

However, the re-examination of the formulation of a coated layer, improvement by means of a press part, or the like is a simple extension of prior art. Even if the technique improves print visual quality, operability and productivity in production premises are not improved, and thus, such a technique is not a basic solution.
Patent Document 1: Japanese Patent Application Laid-Open No. 11-279992
Patent Document 2: Japanese Patent Application Laid-Open No. 11-001891

### Disclosure of the Invention

### Problems to be Solved by the Invention

Therefore, a primary problem of the present invention is to increase productivity and also produce a coated paper with quality required for a coated paper, while a basis weight of a product is decreased to less than 64 g/m² and ultra lightweight coating is performed attributable to reduction in recent paper cost.

Another problem is to obtain a coated paper of good print visual quality having a glossiness of 55% or more, more desirably 60% or more. Still another problem is to be capable of producing a coated paper with high productivity while coping with environmental problems even if a waste paper has a high blend degree of 10% or more. Further problems will be clarified by descriptions below.

### Means for Solving the Problems

The present invention having solved the above problems is defined in process claim 1 and product claim 4. Embodiments of the invention are subject of the dependent claims.

### Advantage of the Invention

According to the present invention, a brilliant high-quality coated paper can be produced at a high production efficiency even for a base paper with low grams per square meter and high blending of a waste paper. The advantage of the present invention is clarified by examples and comparative examples that have been diligently studied for a long period of time and are described below.

A high quality coated paper excellent in glossiness, smoothness, printing suitability, etc., can be produced, with extremely good operationability being secured, in high speed paper making at a paper making speed of exceeding 1300 m/min by means of a process for producing a coated paper according to the present invention using paper making equipment (online machine) integratedly from a paper raw material to a product.

The present invention is intended to produce, for example, a coated paper or ultra lightweight coated paper having 10% or more of a waste paper blended in its raw material as a raw material pulp, with paper grams per square meter of from 28 to 80 g/m² (particularly from 35 to 48 g/m²), product grams per square meter of from 30 to 103 g/m² (particularly from 35 to 64 g/m²) and a one-side coating amount of from 2 to 23 g/m² (particularly from 4 to 9 g/m²) continuously and integratedly from paper making to winding at a paper making speed of 1300 m/min or more, for example, at a high speed of an average paper making speed of from 1600 m/min to 1800 m/min. In addition, desirably, the coating amount is from 2 to 10 g/m² (particularly from 5 to 7 g/m²) at one side in roll coating, and from 6 to 15 g/m² (particularly from 7 to 9 g/m²) at one side in blade coating. Usually, both-face coating is desirably carried out, and thus the amount is twice the above one-side coating amount.

The present invention can make the number of operators smaller. In re-reeler equipment of re-reeling and off-calender requiring running termination and paper joining, a total of 16 operators (4 groups (each 4 operators) and three shifts) are generally required. However, the present invention can remove the 16 operators.

### Best Mode for Carrying Out the Invention

Next, a best mode for carrying out the present invention will be described with reference to the drawings and further the present invention will be set forth in detail.
Referring to FIG. 1, a paper making machine is placed in which a paper is made by a gap type twin wire former 10 for forming a paper layer by ejecting a paper material J from a head box 3 into between two wires (a first wire 1 and a second wire 2) each of which loops. The paper material J is ejected into between a suction (forming) roll 4A and a roll 4B facing each other and between the wires in the wire part thereby to form a paper layer. The paper layer is dewatered to, for example, about a raw material concentration of about 20% while passing through the suction (forming) 4A, a blade 5, a suction couch roll 6, a suction box 7, etc.

Here, a combination use form of roll means and blade dewatering means in the illustration shown is indicated as a dewatering mechanism, and preferably the both are used, but only one is possibly used.

The head box 3 is in a vertical or downstream inclined state and upward disposed. As enlargedly shown in FIG. 6, an ejection angle θ which the paper material ejection direction line makes the horizontal line is desirably from 50° to 90°. In high speed paper making intended by the present invention, an upward head box in which the influence of the fiber weight is small is desirable from the viewpoints of texture, the Z axis strength, front and back difference, fiber orientation angles, etc. In a gap type twin wire former, when the head box is horizontal or the like, desirable propertie's are difficult to obtain in high speed paper making.

A paper layer in the wire part moves to the press part and further dewatered. The press part in an embodiment, in which a first press 21 and a second press 22 respectively have shoe presses 21a, 22a, is made to be a configuration in which a paper layer is straightly nipped to remove open draw and prevent paper breakage. In addition, a belt in the second press 22 is placed on the bottom side relative to the first press 21 of a double felt, and the press is configured so as to prevent wetting again and improve dewatering. Where the basis weight is as high as 60 g/m² or more and the amount of dewatering is large, a double felt is desirable.

A wet paper of a moisture of about 50% having passed through the press part, as referred to FIG. 2, moves to a pre-dryer part of a single deck system and is dried. An illustrated dryer part is a single deck dryer of no open draw system and is configured so as to include an appropriate number of rolls, with the upper side being a heating roll 31 and the lower side being a vacuum roll 32. A single deck dryer has little paper breakage in high speed paper making at 1300 m/min or more that is a target of the present invention, can perform drying at a high efficiency and is excellent in quality and operation. Although a system can be taken into account in which a double deck system is used for drying, it poses problems from the viewpoints of operation properties such as canvas marks in high speed paper making, paper breakage in high speed drying, cockles and paper joining.

In the initial period in a dryer, desirably, partitioned groups are made many for draw adjustment and a suction box 33 is disposed for improvement of air passing through paper and sheet traveling.

A paper web dried in the pre-dryer part, as shown in FIG. 3, is coated with a sizing agent such as starch and, as required, an undercoating liquid such as a pigment coating liquid in a size press 40 of a film transfer (system) between the pre-dryer part and an after dryer part. The size press 40 accepts a gate roll coater 40A or the like, in addition to an illustrated rod metaling size pre-coater.

The undercoating liquids that can be used include, besides starch as mentioned above, starch derivatives such as oxidized starch, estrified starch, enzyme-modified starch and etherified starch, and natural adhesives such as soy bean protein, yeast protein and cellulose derivatives. As required, a pigment may be added thereto. The pigments include kaolin, clay, barium sulfate, light calcium carbonate, heavy calcium carbonate, aluminum hydroxide, satin white, titanium dioxide, calcium sulfite, zinc sulfate, and plastic pigments. The pigment, a usual pigment for a coated paper, is blended depending on respective pigment properties. Moreover, the adhesives that can be used include usual additives for a coated paper including synthetic resin adhesives such as alkali non-sensitive or alkali sensitive synthetic resin emulsions, for example, conjugated diene copolymer latexes such as styrene/butadiene copolymers and methylmethacrylate/butadiene copolymers, acrylic polymer latexes such as polymers or copolymers of acryl and/or methacrylate esters and vinyl acetate copolymer latexes such as ethylene/vinyl acetate copolymers. As required, a variety of assistants can be blended that include a dispersing agent, a flow-modified agent, an anti foaming agent, a dye, a lubricant, a water resistant additive and a water retention agent. The coating amount of a base coating agent is preferably from 0.01 to 4 g/m², particularly preferably from 0.2 to 3 g/m².

Examples of the coating means of a film transfer system that can be used include a gate roll coater, a sim sizer, and a blade metaling size press or a rod metaling size press. Particularly desired is a rod metaling size press. When this rod metaling size press coater is employed, a rod having a smooth surface is desirably used to avoid streak generation in operation. Setting the rod diameter to be from 15 to 50 mm can obtain more preferable operation properties and quality. A rod having a diameter of less than 15 mm is liable to lead to decreasing in film forming capability and becoming inferior in surface. For a rod having a diameter of more than 50 mm, the effect is not changed, and thus a particularly large diameter is not required. A rod with a groove, a rod winding a wire therearound, or the like can be also used as the rod.

After coating of an undercoating liquid, an auxiliary drying device 42 using an air turn bar 41 and an infrared ray is desirably disposed in advance in an after dryer part in order to avoid the generation of surface dirt.

In the illustrated after dryer part of a single deck, a sizing agent and a pigment coating liquid are dried.

Thereafter, in a coater part, an aqueous coating liquid having an additive and a pigment (clay or the like) as primary components is applied. In this case, roll-coating an aqueous coating liquid is adopted from the viewpoint of the quality of the resulting coated paper because a flat coated layer is required, at a paper making speed of 1300 m/min or more so as not to generate paper breakage and not to generate paper breakage in a second blade coating apparatus.

As such, prior to roll coating of an aqueous coating liquid, a surface coated with a sizing agent is desirably flattened by a pre-calender 50 in order to secure higher smoothness. The pre-calender 50 of the embodiment has a metal roll 51 on an upper side and an elastic roll 52 on a lower side.

In operation conditions in the pre-calender 50, a heat roll instead of a metal roll is desirable. Desirably, the temperature is set at, for example, from 100 to 300°C, particularly from 150 to 250°C, and the linear pressure is set at 50 KN/m. Both the rolls can be metal rolls and further a caliper control roll can also be used in order to control the profile in the width direction.

A coater part of the present invention subsequent to the pre-calender 50 has a first roll coating step to both the faces of a paper to be coated and a second blade coating step to both the faces of a paper to be coated and selectively carries out coating.

In other words, when passed through the first roll coating step, the paper to be coated is coated on its both faces by a roll coater 60. After passed through an air turn bar 61, the resulting paper, in the width direction, is dried by a temperature controllable auxiliary drying device 62 using an infrared ray (having the same function as in other cases), a first gas-type air dryer 63A, an infrared ray auxiliary drying device 63A, an infrared ray auxiliary drying device 67A and a first canvas dryer 64. Thereafter, the resulting paper is passed through a bypass pathway Y, dried by a second canvas dryer 68, and then led to a calender 70.

Where passed through the second blade coating step, the paper is passed through the pre-calender 50 and then through a bypass pathway X. The paper is, without being passed through the roll coater, directly led to a first blade coater 65A, where one face of the paper is coated. After coated, the paper is dried by an infrared ray auxiliary drying device 66A, the first gas-type air dryer 63A, the infrared ray auxiliary drying device 67A and the first canvas dryer 64.

Thereafter, the paper is, without being passed through the bypass pathway Y, led to a second blade coater 65B, where the other face is coated. After coated, the resulting paper is dried by an infrared ray auxiliary drying device 66B, a second gas-type air dryer 63B, an infrared ray auxiliary drying device 67B and the second canvas dryer 68, and led to a calender 70.

Where, the paper to be coated is subjected to lower layer coating on its both faces by the roll coater 60 via a bypass pathway Z and can also be subjected to upper layer coating by use of the first blade coater 65A and the second blade coater 65B.

The above-mentioned infrared ray auxiliary drying devices can be used for temperature control in the width direction in order to mainly each adjust moisture contents, and their adoption can be selected as appropriate.

In the first blade coater 65A and the second blade coater 65B, a coating amount of 7 g/m² or more per face may be required in the case of high speed paper making. In such a case, a jet fountain system capable of making high speed liquid provision as an applicator is desirable and raking off is made by a blade. When a coating amount of less than 7 g/m² for one face is required, a short dwell blade coater improved for high speed is also acceptable.

In blade coating, as shown in FIG. 10, a fountain angle α of an applicator 90 in the case where the coating of a jet fountain system is adopted from 30 to 90 degrees, more desirably from 40 to 60 degrees, in order to remove coating unevenness in the flow and width directions for roll coating. When the fountain angle α is out of the above range, a rough surface and coating unevenness are generated. A system having a bevel angel θ of from 30 to 50 degrees in a blade edge is desirable. The thickness of a blade is desirably from 0.45 to 0.60 mm. For the possession of a high hardness, the blade edge is constituted by a thermal spraying material having tungsten or alumina oxide as a primary component. For example, a system, having excellent conditions in coating properties, has a constitution produced by thermally spraying tungsten to a base material making up the edge of a blade and has a Vickers hardness of from 1000 to 1700 Hv.

In this case, after blade exchange, cooling means such as water shower cooling is desirably disposed to prevent blade burning at a high speed paper making at a time of new blade touch.

Finally, an on-machine calender 70 constituted by a thermal soft calender is disposed and calender treatment is implemented. The illustrated calender 70 is a multiple calender of one stack type of 9 nips of vertical placement of an optiload type. One stack type of 7 nips can also be used and also Janus type inclined placement, illustrated together, that makes the influence of roll deadweight small is allowable.

The calender 70 affects final smoothness and glossiness. Hence, a variety of considerations are required in terms of this and high speed paper making.

The number of stages of the calender 70 is not limited so long as the calender has at least two nips, and a flattening treatment is desirably implemented by a thermal soft calender comprising a combination of a metal roll M and an elastic roll D formed in a multi-stage. In particular, a multi-nip calender, more desirably a multi-nip calender of 6, 8 or 10 stages is most suitable.

On the other hand, a thermal calender may be a calender in which a thermal medium such as oil is circulated and heated, but this has a limit of a surface temperature of about 180°C. For the implementation of paper making at a high speed, as shown in FIGS. 7 to 9, the metal roll M includes an internal heating device having electromagnetic induction action capable of split temperature control in its width direction, and treatment is desirably carried out at a surface temperature of the metal roll M of 230°C or more, particularly from 230 to 500°C. A specific example is a roll in which an induction coil 71 is wound around an iron core 72 within a shell 74 and a heat medium passed through a jacket chamber 73 is heated.

A surface treatment is performed at a temperature of from 250°C to 380°C of the metal roll M, particularly at a temperature of from 300°C exclusive to 380°C inclusive, and a paper is not broken throughout the entire layer at as low a nip pressure as possible to be capable of preventing a decrease in bulk and of restraining a decrease in opacity, whereby operation can also be implemented. In short, it is a mode in which an iron at an extremely high temperature is contacted for a short time.

The methods of controlling the surface temperature of a metal roll that are particularly excellent for elevated temperature treatment of the present invention include, in addition to a method of circulating hot water or oil into a metal roll, as described above, a method by an "internal heating device by electromagnetic induction action" that involves disposing an induction coil around an iron core disposed in an inside as a non-rotation portion, flowing an alternating current into its induction coil to generate a magnetic flux in the coil and induce an induction current inside an external shell (external cylinder) as a rotation portion and self heat releasing (induction heat release) the outside shell (external cylinder) by its resistance heat. In addition, according to the internal heating device by the electromagnetic induction action, there is an advantage that an induction coil is divided (e.g., 3 to 6 divisions) in the width direction (longitudinal direction of the roll itself) and an alternating current amount flowed into a corresponding induction coil is controlled based on a temperature signal from a temperature sensor disposed in the shell, so that the temperature control in the width direction particularly on the surface is possible at high precision.

In this case, a structure in which jacket pathways particularly extended in the longitudinal direction inside the shell are disposed in large numbers, from 10 to 90 pathways, in the peripheral direction at intervals, in which these are connected to each other, and in which a heat medium is enclosed in the inside, is more excellent from the viewpoints of heat due to self heat releasing of the shell being absorbed and the heat being uniformed on the entire roll surface.

A surface treatment at elevated temperature according to the present invention increases not only the temperature of the surface layer portion of a paper but the temperature of the inner layer portion. As a result, not only the surface layer portion of the paper but the entire layer is liable to break, so that the bulk is lowered. Therefore, where a paper is passed for a short time by further high temperature treatment, heat transfer to the inner layer portion can be prevented extremely, thereby being capable of preventing a decrease in bulk.

On the contrary, with increased temperature of the surface temperature of a metal roll, the stress in the width direction in the shell of a metal roll is generated and the roll profile is likely to be destroyed, whereby the controlling of a thick paper profile is decreased. In addition, when a metal roll depends on an internal heating device by electromagnetic induction action, the temperature response of the surface temperature of the metal roll per time does not seem to be good. Moreover, due to this, the temperature response in the width direction is bad, which is a cause of yield decrease because of bad temperature controlling. Thus, at least either an external heating device by electromagnetic induction action capable of division temperature control in the roll width direction or a cooling apparatus capable of cooling temperature control in the roll width direction is desirably provided in the vicinity of the metal roll M.

This example will be primarily described in reference to FIG. 8. The metal roll M includes a shell 74, an induction coil 71, an iron core 72, a temperature sensor 75, an alternating current source 76 and a jacket pathway 73. With this metal roll M, an internal heating device 77 by electromagnetic induction action capable of division temperature control in the roll width direction is disposed in the vicinity of the metal roll M to constitute a high temperature nip region of a base paper.

The internal heating device 77 is an application of the principle of electromagnetic induction heating. As shown in the drawing, the internal heating device 77 entails flowing an alternating current (e.g. , a high frequency of from 3 to 20 kHz) from an alternating current source (inverter) 77B to a work coil 77A to generate a magnetic field, generating an eddy current on a shell 74 surface portion, and self heat releasing. The separation distance between the work coil 77A and the shell 74 surface is desirably from 2 to 20 mm, particularly desirably roughly from 2 to 5 mm. In addition, a unit work coil is desirably inclination-disposed so as to cross the shaft of the metal roll M for the purpose of texture of a profile for heating purposes. The zone control pitch in the roll width direction is roughly from 75 to 150 mm, and the rating electric power per zone can be set at from 4 to 20 kW.

An example of a cleaning apparatus 78 capable of cooling temperature control in the roll width direction is as follows. As shown in FIG. 9, air is sent from a fan 78a to a header 78b and the air is sent into a temperature adjusting chamber 78d through an adjusting plate 78c having communicated pores formed therein. Then, a coil 78e disposed within the temperature adjusting chamber 78d is cooled by temperature adjusting means 78f to control the ventilation temperature passing through a dispersion plate 78g having small pores.

The nip pressure in the calender 70 is desirably from 200 KN/m to 450 KN/m, particularly desirably from 300 KN/m to 450 KN/m. The paper flattening treated by the calender 70 is finally wound by a reel 80, and a winder (not shown) for finishing winding for subdivision is disposed in the final portion of the machine.

In place of the multi-nip calender shown in FIG. 4, as illustrated in FIG. 5, for example, a soft calender 70A including the metal roll M constituted by 1 nip and 4 stacks and the elastic roll D is acceptable.

### EXAMPLES

Advantages of the present invention will be clarified by means of examples and comparative examples.
Factors such as a wire part mode, a placement angle of the head box, a suction mode, a coating mode, a thermal soft calender and a paper making speed, of the present invention, were changed and quality of paper were evaluated. In addition, each of the examples did not newly dispose individual lines for each of all the factors and testing examples by testing plants were primarily newly replaced.

Quality evaluations of paper are in the following.
1. Contaminants: The area of contaminants was evaluated by connecting a CCD camera to an optical microscope and measuring one sheet A4 paper at a magnification of 8 µm per pixel via an image analyzing unit (LUZEX AP) and then averaging them for 10 cm². In addition, contaminants of 0.005 mm² or less could not visually be recognized, and thus were neglected.
2. Texture evaluation: The texture evaluation stipulated in the example was implemented by obtaining the variation of a transmitted light amount as a time sequence signal using a sheet texture tester available from TOYO SEIKI KOGYO CO., LTD. This measuring device can measure 28 points in the wavelength range of unevenness of from about 0.16 to about 80 mm. However, because 14 points in the range of from 4.0 to 80 mm in the example were closely related to texture indicated by large shades in watermark texture by sensory inspection, the sum of the coefficients of variation in the range was determined. When the unevenness index is less than 6%, the texture is very in uniform, the glossiness unevenness of a coated paper surface attributable to texture unevenness hardly occurs, the formation of a coated layer is uniform, and printing unevenness at printing, printing glossiness unevenness, etc. disappear, so that printing suitability is improved.
3. Paper breakage: A test operation was conducted at a paper making speed of 1500 m/min at a constant drying temperature for 3 hours using a test plant equivalent to an actual machine and the number of paper breaks due to the difference of drying methods was evaluated.
   ○ : Number of paper breaks, 0 time; Δ: one time; × : one or more times.
4. Cockle: A test operation was conducted at a paper making speed of 1300 m/min at a constant drying temperature for 3 hours using a test plant and the number of cockles due to the difference of drying methods was evaluated. ○: Number of cockles, 0; Δ: one; ×: one or more.
5. Specific volume: Measured in accordance with JIS P 8118 (1976).
6. Glossiness: Was measured at an angle of 75 degrees in accordance with JIS P 8142.
7. Glossiness unevenness: Test paper sheets of an A4 size were prepared, and were visually evaluated by five females and five males on the basis of five criteria. Level 3 or higher was regarded allowable.
8. Printing unevenness: Test paper sheets of a duodecimo size were prepared, and printed using a Rowland offset printer, left to stand for 24 hours at a constant temperature. Then, solid printed portions of samples, overprinted with four colors of black, magenta, cyan and yellow, were visually evaluated by five females and five males on the basis of five criteria. Level 3 or higher was regarded allowable.
9. Rigidity: Determined in accordance with JIS P 8115.
10. Yellow change (by calender treatment) : A product was prepared to a duodecimo size and the extent of yellow of the product was visually evaluated by five females and five males on the basis of five criteria. Level 3 or higher was regarded allowable.
11. Productivity: stability of a wet end, dewater properties in a press part, generation states of drainage and streaks, etc. in each example in a test machine were observed by five operators, and each of the evaluation results was collected and evaluated based on 5 criteria. Level 3 or higher was regarded allowable.
12. Overall evaluation: All of the quality attributes were all totally evaluated on the basis of four criteria. ⊚: Good production efficiency/quality, ○: No problems in production efficiency/quality, Δ: Some problems, ×: Problems.
In addition, the roll hardness of a roll coater is the A hardness value of JIS K 6301, and the hardness of a blade is the Hv (hard Vickers). The roll surface roughness indicates the central line average roughness in accordance with JIS P 0601.

Base paper conditions are as follows:

### <Production of paper base material>

A base paper having pulp below and a basis weight (absolute dry) of 60 g/m² was made to produce a paper base material.

### <Blending of pulp>

A pulp was prepared according to the example tables. In the present invention, paper breakage was frequently generated due to the affect of contaminants in high speed paper making. For this reason, a raw material pulp was prepared such that the amount of contaminants in a product was 0.010 mm²/10 cm² or less per A4 size sheet in the measuring amount in contaminant measuring means and used.
A paper base material was prepared using the above pulp blending and the internal additive agent blending below.

### <Blending of internal additive agents>

- Soft calcium carbonate: 10 weight parts (average particle diameter: 3.4 µ, calcite-based)
- Commercially available alkylketene dimmer-based internal sizing agent (AKD): 0.03 weight part
- Commercially available cationized starch: 0.2 weight part
- Commercially available cation-based polyacrylamide yield improving agent: 0.03 weight part

### <Size press>

A starch coating liquid was applied in an amount of 0.5 g/m² onto the above paper base material and dried.

### <Production of coated paper>

The coating liquid having the blend below was applied onto a paper base material after the above size press using a roll coater and a blade coater according to examples and dried.

### <Blending of overcoating liquid>

Blending is as follows:

### (Pigments)

- Spindle-shaped soft calcium carbonate (TPI121 available from OKUTAMA KOGYO CO., LTD., 3.4 µm): 30 weight parts
- Commercially available fine particle kaolin (Amazon 88, average particle diameter: 0.8 µm) : 70 weight parts

### (Binders and additives)

- Commercially available phosphoric acid esterified starch (MS4400 available from NIHON SHOKUHIN KAKO CO. , LTD.) : 1 weight part
- Styrene/butadiene latex (0617 available from JSR CORPORATION): 12 weight parts
- Commercially available polyacrylic acid-based dispersing agent: 0.1 weight part
- Commercially available calcium stearate: 0.3 weight part
- Sodium hydroxide: 0.15 weight part

Under the conditions above and the conditions indicated - in Tables, a variety of factors were searched and the results listed in Tables 1 to 36 were obtained. Examples 1 to 42 indicate examples of a combination of roll coating and blade coating only, Examples 43 to 56 indicate examples of roll coating only, and Examples 57 to 69 indicate examples of blade coating only.

**[Table 1]**

| | Wet paper forming step | | | Press part (1 P) | | Blade dryer | Size press | After dryer | Pre-calender | Paper making speed |
|---|---|---|---|---|---|---|---|---|---|---|
| | Wire part mode | Suction mode | | | | | | | Soft calender | |
| | | 1 Stage | 2 Stage | Mode | Felt constitution | Mode | Mode | Mode | Mode | m/min |
| Example 1 | Gap former | Suction roll | Suction blade | Shoe press | Double felt | Single deck | Gate roll | Single deck | 1 Nip 1 stack | 1300 |
| Example 2 | Gap former | Suction roll | Suction blade | Shoe press | Double felt | Single deck | Gate roll | Single deck | 1 Nip 1 stack | 1400 |
| Example 3 | Gap former | Suction roll | Suction blade | Shoe press | Double felt | Single deck | Gate roll | Single deck | 1 Nip 1 stack | 1600 |
| Example 4 | Gap former | Suction blade | Suction roll | Shoe press | Double felt | Single deck | Gate roll | Single deck | 1 Nip 1 stack | 1800 |
| Example 5 | Gap former | Suction roll | Suction roll | Shoe press | Double felt | Single deck | Gate roll | Single deck | 1 Nip 1 stack | 1400 |
| Example 6 | Gap former | Suction blade | Suction blade | Shoe press | Double felt | Single deck | Gate roll | Single deck | 1 Nip 1 stack | 1600 |
| Example 7 | Gap former | Suction roll | Suction blade | Shoe press | Double felt | Single deck | Gate roll | Single deck | 1 Nip 1 stack | 1400 |
| Example 8 | Gap former | Suction roll | Suction blade | Shoe press | Double felt | Single deck | Rod metaling | Single deck | 1 Nip 1 stack | 1600 |
| Comparative Example 1 | Gap former | Suction roll | Suction blade | Press | Single felt | Double deck | - | Single deck | 1 Nip 1 stack | 1000 |
| Comparative Example 2 | Gap former | Suction roll | Suction blade | Press | Single felt | Double deck | - | Double deck | - | 1100 |
| Comparative Example 3 | Long net | Suction blade | - | Shoe press | Double felt | Single deck | - | Single deck | - | 1200 |
| Comparative Example 4 | Gap former | Suction roll | - | Press | Single felt | Single deck | - | Double deck | - | 1400 |
| Comparative Example 5 | Long net | Suction blade | - | Shoe press | Double felt | Single deck | - | Double deck | - | 1100 |
| Comparative Example 6 | Gap former | Suction roll | Suction blade | Press | Single felt | Double deck | - | Double deck | - | 1100 |
| Comparative Example 7 | Gap former | Suction blade | Suction roll | Press | Single felt | Double deck | - | Double deck | 1 Nip 1 stack | 1100 |

**[Table 2]**

| | First coating apparatus | | | | Coating amount |
|---|---|---|---|---|---|
| | Coater mode | Hardness | Roll surface roughness | Material | Both faces |
| | | Hv | µm | | g/m² |
| Example 1 | Roll | 70 | 5 | Urethane coated roll | 10 |
| Example 2 | Roll | 75 | 5 | Polyether resin coated roll | 10 |
| Example 3 | Roll | 80 | 5 | Polyethylene blended urethane roll | 10 |
| Example 4 | Roll | 85 | 5 | Urethane coated roll | 10 |
| Example 5 | Roll | 90 | 5 | Polyethylene blended urethane roll | 10 |
| Example 6 | Roll | 80 | 10 | Urethane coated roll | 10 |
| Example 7 | Roll | 80 | 5 | Urethane coated roll | 10 |
| Example 8 | Roll | 80 | 2 | Urethane coated roll | 10 |
| Comparative Example 1 | Blade/blade | 1100 | - | Tungsten | 10 |
| Comparative Example 2 | Blade/blade | 1100 | - | Alumina oxide | 10 |
| Comparative Example 3 | Roll | 70 | 5 | Urethane coated roll | 10 |
| Comparative Example 4 | Blade/blade | 900 | - | Tungsten carbide | 10 |
| Comparative Example 5 | Roll | 70 | 5 | Urethane coated roll | 10 |
| Comparative Example 6 | Blade/blade | 1400 | - | Tungsten | 10 |
| Comparative Example 7 | Blade/blade | 1100 | - | Tungsten | 10 |

**[Table 3]**

| | Second coating apparatus (Front) | | | | | | |
|---|---|---|---|---|---|---|---|
| | Coating mode | Mode | Material | Thickness | Hardness | Bevel angle | Fountain angle |
| | | | | mm | Hv | | Degree |
| Example 1 | Jet fountain | Blade | Tungsten | 0.6 | 1400 | 40 | 50 |
| Example 2 | Jet fountain | Blade | Tungsten | 0.6 | 1400 | 40 | 50 |
| Example 3 | Jet fountain | Blade | Tungsten | 0.6 | 1400 | 40 | 50 |
| Example 4 | Jet fountain | Blade | Tungsten | 0.5 | 1000 | 30 | 50 |
| Example 5 | Jet fountain | Blade | Tungsten | 0.7 | 1400 | 50 | 50 |
| Example 6 | Jet fountain | Blade | Tungsten | 0.5 | 1600 | 40 | 50 |
| Example 7 | Jet fountain | Blade | Alumina oxide | 0.6 | 1400 | 40 | 45 |
| Example 8 | Jet fountain | Blade | Tungsten | 0.6 | 1400 | 40 | 60 |
| Comparative Example 1 | Jet fountain | Blade | Tungsten | 0.4 | 900 | 40 | 25 |
| Comparative Example 2 | Jet fountain | Blade | Tungsten | 0.5 | 900 | 40 | 25 |
| Comparative Example 3 | Applicator roll | Roll coater | - | - | - | - | - |
| Comparative Example 4 | Jet fountain | Blade | Tungsten | 0.5 | 900 | 40 | 25 |
| Comparative Example 5 | Applicator roll | Roll coater | - | - | - | - | - |
| Comparative Example 6 | Jet fountain | Blade | Tungsten | 0.4 | 1500 | 65 | 50 |
| Comparative Example 7 | Jet fountain | Blade | Tungsten | 0.5 | 900 | 40 | 25 |

**[Table 4]**

| | Second coating apparatus (Back) | | | | | | | Coating amount |
|---|---|---|---|---|---|---|---|---|
| | Coating mode | Mode | Material | Thickness | Hardness | Bevel angle | Fountain angle | Product coating amount |
| | | | | mm | Hv | | Degree | g/m² |
| Example 1 | Jet fountain | Blade | Tungsten | 0.6 | 1400 | 40 | 50 | 24 |
| Example 2 | Jet fountain | Blade | Tungsten | 0.6 | 1400 | 40 | 50 | 24 |
| Example 3 | Jet fountain | Blade | Tungsten | 0.6 | 1400 | 40 | 50 | 24 |
| Example 4 | Jet fountain | Blade | Tungsten | 0.5 | 1000 | 30 | 50 | 24 |
| Example 5 | Jet fountain | Blade | Tungsten | 0.7 | 1400 | 50 | 50 | 24 |
| Example 6 | Jet fountain | Blade | Tungsten | 0.5 | 1600 | 40 | 50 | 24 |
| Example 7 | Jet fountain | Blade | Alumina oxide | 0.6 | 1400 | 40 | 60 | 24 |
| Example 8 | Jet fountain | Blade | Tungsten | 0.6 | 1400 | 40 | 45 | 24 |
| Comparative Example 1 | Jet fountain | Blade | Tungsten | 0.4 | 900 | 40 | 25 | 24 |
| Comparative Example 2 | Jet fountain | Blade | Tungsten | 0.5 | 900 | 40 | 25 | 24 |
| Comparative Example 3 | Applicator roll | Roll coater | - | - | - | - | - | 24 |
| Comparative Example 4 | Jet fountain | Blade | Tungsten | 0.5 | 900 | 40 | 25 | 24 |
| Comparative Example 5 | Applicator roll | Roll coater | - | - | - | - | - | 24 |
| Comparative Example 6 | Jet fountain | Blade | Tungsten | 0.4 | 1500 | 65 | 50 | 24 |
| Comparative Example 7 | Applicator roll | Roll coater | Tungsten | - | - | - | - | 24 |

**[Table 5]**

| | Flattening treatment step | | | | Product grams per square meter | Raw material | | | Contaminant amount |
|---|---|---|---|---|---|---|---|---|---|
| | Stage number | Temperature | Surface roughness | Elastic roll hardness | | Waste paper | NBKP | LBKP | |
| | | °C | µm | Hv | g/m² | % | % | % | |
| Example 1 | 9 | 140 | 3 | 90 | 54.2 | 20 | 60 | 20 | 0.086 |
| Example 2 | 9 | 140 | 3 | 95 | 54.2 | 20 | 60 | 20 | 0.077 |
| Example 3 | 9 | 140 | 3 | 98 | 54.2 | 20 | 60 | 20 | 0.085 |
| Example 4 | 9 | 140 | 2.5 | 97 | 54.2 | 20 | 60 | 20 | 0.083 |
| Example 5 | 9 | 140 | 4.5 | 97 | 54.2 | 20 | 60 | 20 | 0.073 |
| Example 6 | 9 | 140 | 3 | 97 | 54.2 | 20 | 60 | 20 | 0.075 |
| Example 7 | 9 | 130 | 3 | 97 | 54.2 | 20 | 60 | 20 | 0.080 |
| Example 8 | 9 | 180 | 3 | 97 | 54.2 | 20 | 60 | 20 | 0.074 |
| Comparative Example 1 | 9 | 140 | 2 | 88 | 54.2 | 20 | 60 | 20 | 0.084 |
| Comparative Example 2 | 9 | 140 | 2 | 95 | 54.2 | 20 | 60 | 20 | 0.070 |
| Comparative Example 3 | 9 | 140 | 2 | 95 | 54.2 | 20 | 60 | 20 | 0.086 |
| Comparative Example 4 | 9 | 120 | 3.5 | 88 | 54.2 | 20 | 60 | 20 | 0.073 |
| Comparative Example 5 | 9 | 180 | 5 | 88 | 54.2 | 20 | 60 | 20 | 0.087 |
| Comparative Example 6 | 1 nip | 120 | 2 | 95 | 54.2 | 20 | 60 | 20 | 0.070 |
| Comparative Example 7 | 1 nip | 160 | 3.5 | 95 | 54.2 | 20 | 60 | 20 | 0.080 |

**[Table 6]**

| | Quality evaluation | | | | | | | | | | |
|---|---|---|---|---|---|---|---|---|---|---|---|
| | Texture | Paper breakage | Cockle | Specific volume | Glossiness | Glossiness unevenness | Printing unevenness | Rigidity | Yellow change | Productivity | Overall evaluation |
| Example 1 | 5.7 | ○ | ○ | 1.17 | 60 | 4 | 4 | 65 | 5 | 4 | ○ |
| Example 2 | 5.6 | ○ | ○ | 1.18 | 60 | 4 | 4 | 66 | 5 | 5 | ○ |
| Example 3 | 5.6 | ○ | ○ | 1.17 | 62 | 5 | 4 | 65 | 5 | 4 | ⊚ |
| Example 4 | 5.6 | ○ | ○ | 1.17 | 61 | 4 | 4 | 67 | 5 | 4 | ○ |
| Example 5 | 5.6 | ○ | ○ | 1.18 | 61 | 5 | 5 | 65 | 5 | 4 | ⊚ |
| Example 6 | 5.6 | ○ | ○ | 1.18 | 58 | 4 | 4 | 66 | 5 | 4 | ○ |
| Example 7 | 5.6 | ○ | ○ | 1.18 | 60 | 4 | 4 | 67 | 5 | 4 | ○ |
| Example 8 | 5.6 | ○ | ○ | 1.18 | 60 | 4 | 4 | 64 | 4 | 4 | ○ |
| Comparative Example 1 | 5.6 | Δ | Δ | 1.17 | 53 | 3 | 4 | 42 | 3 | 1 | Δ |
| Comparative Example 2 | 5.6 | × | × | 1.16 | 54 | 3 | 4 | 43 | 3 | 2 | × |
| Comparative Example 3 | 5.2 | ○ | × | 1.18 | 52 | 1 | 1 | 48 | 3 | 2 | × |
| Comparative Example 4 | 5.4 | × | × | 1.18 | 53 | 2 | 3 | 44 | 4 | 3 | × |
| Comparative Example 5 | 5.2 | ○ | Δ | 1.17 | 52 | 1 | 1 | 47 | 1 | 2 | × |
| Comparative Example 6 | 5.5 | × | × | 1.13 | 40 | 2 | 2 | 45 | 3 | 2 | × |
| Comparative Example 7 | 5.5 | Δ | Δ | 1.18 | 39 | 3 | 3 | 44 | 2 | 2 | × |

**[Table 7]**

| | Wet paper forming step | | | Press part (1 P) | | Pre-dryer | Size press | After dryer | Pre-calender | Paper making speed |
|---|---|---|---|---|---|---|---|---|---|---|
| | Wire part mode | Suction mode | | | | | | | Soft calender | |
| | | 1 Stage | Stage | Mode | Felt constitution | Mode | Mode | Mode | Mode | m/min |
| Example 9 | Gap former | Suction roll | Suction blade | Shoe press | Double felt | Single deck | Gate roll | Single deck | 1 Nip 1 stack | 1600 |
| Example 10 | Gap former | Suction roll | Suction blade | Shoe press | Double felt | Single deck | Gate roll | Single deck | 1 Nip 1 stack | 1600 |
| Example 11 | Gap former | Suction roll | Suction blade | Shoe press | Double felt | Single deck | Gate roll | Single deck | 1 Nip 1 stack | 1600 |
| Example 12 | Gap former | Suction roll | Suction blade | Shoe press | Double felt | Single deck | Gate roll | Single deck | 1 Nip 1 stack | 1600 |
| Example 13 | Gap former | Suction roll | Suction blade | Shoe press | Double felt | Single deck | Gate roll | Single deck | 1 Nip 1 stack | 1600 |
| Example 14 | Gap former | Suction roll | Suction blade | Shoe press | Double felt | Single deck | Gate roll | Single deck | 1 Nip 1 stack | 1600 |
| Example 15 | Gap former | Suction roll | Suction blade | Shoe press | Double felt | Single deck | Gate roll | Single deck | 1 Nip 1 stack | 1600 |
| Example 16 | Gap former | Suction roll | Suction blade | Shoe press | Double felt | Single deck | Gate roll | Single deck | 1 Nip 1 stack | 1600 |
| Example 17 | Gap former | Suction roll | Suction blade | Shoe press | Double felt | Single deck | Gate roll | Single deck | 1 Nip 1 stack | 1600 |
| Example 18 | Gap former | Suction roll | Suction blade | Shoe press | Double felt | Single deck | Gate roll | Single deck | 1 Nip 1 stack | 1600 |
| Example 19 | Gap former | Suction roll | Suction blade | Shoe press | Double felt | Single deck | Gate roll | Single deck | 1 Nip 1 stack | 1600 |
| Example 20 | Gap former | Suction roll | Suction blade | Shoe press | Double felt | Single deck | Gate roll | Single deck | 1 Nip 1 stack | 1600 |
| Example 21 | Gap former | Suction roll | Suction blade | Shoe press | Double felt | Single deck | Gate roll | Single deck | 1 Nip 1 stack | 1600 |
| Example 22 | Gap former | Suction roll | Suction blade | Shoe press | Double felt | Single deck | Gate roll | Single deck | 1 Nip 1 stack | 1600 |
| Example 23 | Gap former | Suction roll | Suction blade | Shoe press | Double felt | Single deck | Gate roll | Single deck | 1 Nip 1 stack | 1600 |

**[Table 8]**

| | First coating apparatus | | | | Coating amount |
|---|---|---|---|---|---|
| | Coater mode | Hardness | Roll surface roughness | Material | Both faces |
| | | Hv | µm | | g/m² |
| Example 9 | Roll | 80 | 5 | Polyethylene blended urethane roll | 4 |
| Example 10 | Roll | 80 | 5 | Polyethylene blended urethane roll | 6 |
| Example 11 | Roll | 80 | 5 | Polyethylene blended urethane roll | 8 |
| Example 12 | Roll | 80 | 5 | Polyethylene blended urethane roll | 10 |
| Example 13 | Roll | 80 | 5 | Polyethylene blended urethane roll | 6 |
| Example 14 | Roll | 80 | 5 | Polyethylene blended urethane roll | 6 |
| Example 15 | Roll | 80 | 5 | Polyethylene blended urethane roll | 6 |
| Example 16 | Roll | 80 | 5 | Polyethylene blended urethane roll | 5 |
| Example 17 | Roll | 80 | 5 | Polyethylene blended urethane roll | 5 |
| Example 18 | Roll | 80 | 5 | Polyethylene blended urethane roll | 5 |
| Example 19 | Roll | 80 | 5 | Polyethylene blended urethane roll | 5 |
| Example 20 | Roll | 80 | 5 | Polyethylene blended urethane roll | 5 |
| Example 21 | Roll | 80 | 5 | Polyethylene blended urethane roll | 5 |
| Example 22 | Roll | 80 | 5 | Polyethylene blended urethane roll | 5 |
| Example 23 | Roll | 80 | 5 | Polyethylene blended urethane roll | 5 |

**[Table 9]**

| | Second coating apparatus | | | | | | |
|---|---|---|---|---|---|---|---|
| | Coating mode | Mode | Material | Thickness | Hardness | Bevel angle | Fountain angle |
| | | | | mm | Hv | | Degree |
| Example 9 | Jet fountain | Blade | Tungsten | 0.6 | 1400 | 40 | 50 |
| Example 10 | Jet fountain | Blade | Tungsten | 0.6 | 1400 | 40 | 50 |
| Example 11 | Jet fountain | Blade | Tungsten | 0.6 | 1400 | 40 | 50 |
| Example 12 | Jet fountain | Blade | Tungsten | 0.6 | 1400 | 40 | 50 |
| Example 13 | Jet fountain | Blade | Tungsten | 0.6 | 1400 | 40 | 50 |
| Example 14 | Jet fountain | Blade | Tungsten | 0.6 | 1400 | 40 | 50 |
| Example 15 | Jet fountain | Blade | Tungsten | 0.6 | 1400 | 40 | 50 |
| Example 16 | Jet fountain | Blade | Tungsten | 0.6 | 1400 | 40 | 50 |
| Example 17 | Jet fountain | blade | Tungsten | 0.6 | 1400 | 40 | 50 |
| Example 18 | Jet fountain | Blade | Tungsten | 0.6 | 1400 | 40 | 50 |
| Example 19 | Jet fountain | Blade | Tungsten | 0.6 | 1400 | 40 | 50 |
| Example 20 | Jet fountain | Blade | Tungsten | 0.6 | 1400 | 40 | 50 |
| Example 21 | Jet fountain | Blade | Tungsten | 0.6 | 1400 | 40 | 50 |
| Example 22 | Jet fountain | Blade | Tungsten | 0.6 | 1400 | 40 | 50 |
| Example 23 | Jet fountain | Blade | Tungsten | 0.6 | 1400 | 40 | 50 |

**[Table 10]**

| | Second coating apparatus | | | | | | | Coating amount |
|---|---|---|---|---|---|---|---|---|
| | Coating | Mode | Material | Thickness | Hardness | Bevel angle | Fountain angle | Product coating amount |
| | | | | mm | Hv | | Degree | g/m² |
| Example 9 | Jet fountain | Blade | Tungsten | 0.6 | 1400 | 40 | 50 | 12 |
| Example 10 | Jet fountain | Blade | Tungsten | 0.6 | 1400 | 40 | 50 | 18 |
| Example 11 | Jet fountain | Blade | Tungsten | 0.6 | 1400 | 40 | 50 | 20 |
| Example 12 | Jet fountain | Blade | Tungsten | 0.6 | 1400 | 40 | 50 | 22 |
| Example 13 | Jet fountain | Blade | Tungsten | 0.6 | 1400 | 40 | 50 | 20 |
| Example 14 | Jet fountain | Blade | Tungsten | 0.6 | 1400 | 40 | 50 | 22 |
| Example 15 | Jet fountain | Blade | Tungsten | 0.6 | 1400 | 40 | 50 | 24 |
| Example 16 | Jet fountain | Blade | Tungsten | 0.6 | 1400 | 40 | 50 | 14 |
| Example 17 | Jet fountain | Blade | Tungsten | 0.6 | 1400 | 40 | 50 | 14 |
| Example 18 | Jet fountain | Blade | Tungsten | 0.6 | 1400 | 40 | 50 | 14 |
| Example 19 | Jet fountain | Blade | Tungsten | 0.6 | 1400 | 40 | 50 | 14 |
| Example 20 | Jet fountain | Blade | Tungsten | 0.6 | 1400 | 40 | 50 | 14 |
| Example 21 | Jet fountain | Blade | Tungsten | 0.6 | 1400 | 40 | 50 | 14 |
| Example 22 | Jet fountain | Blade | Tungsten | 0.6 | 1400 | 40 | 50 | 14 |
| Example 23 | Jet fountain | Blade | Tungsten | 0.6 | 1400 | 40 | 50 | 14 |

**[Table 11]**

| | Flattening treatment step | | | | Product grams per square meter | Raw material | | | Contaminant amount |
|---|---|---|---|---|---|---|---|---|---|
| | Stage number | Temperature | Surface roughness | Elastic roll hardness | | Waste paper | NBKP | LBKP | |
| | | °C | µm | Hv | g/m² | % | % | % | |
| Example 9 | 9 | 140 | 3 | 98 | 54.2 | 20 | 60 | 20 | 0.070 |
| Example 10 | 9 | 140 | 3 | 98 | 54.2 | 20 | 60 | 20 | 0.078 |
| Example 11 | 9 | 140 | 3 | 98 | 54.2 | 20 | 60 | 20 | 0.075 |
| Example 12 | 9 | 140 | 3 | 98 | 54.2 | 20 | 60 | 20 | 0.078 |
| Example 13 | 9 | 140 | 3 | 98 | 54.2 | 20 | 60 | 20 | 0.085 |
| Example 14 | 9 | 140 | 3 | 98 | 54.2 | 20 | 60 | 20 | 0.088 |
| Example 15 | 9 | 140 | 3 | 98 | 54.2 | 20 | 60 | 20 | 0.084 |
| Example 16 | 9 | 140 | 3 | 98 | 54.2 | 10 | 60 | 30 | 0.068 |
| Example 17 | 9 | 140 | 3 | 98 | 54.2 | 20 | 50 | 30 | 0.082 |
| Example 18 | 9 | 140 | 3 | 98 | 54.2 | 30 | 40 | 30 | 0.083 |
| Example 19 | 9 | 140 | 3 | 98 | 54.2 | 40 | 30 | 30 | 0.088 |
| Example 20 | 9 | 140 | 3 | 98 | 54.2 | 50 | 30 | 20 | 0.092 |
| Example 21 | 9 | 140 | 3 | 98 | 54.2 | 60 | 30 | 10 | 0.093 |
| Example 22 | 9 | 140 | 3 | 98 | 54.2 | 70 | 30 | - | 0.095 |
| Example 23 | 9 | 140 | 3 | 98 | 54.2 | 100 | - | - | 0.098 |

**[Table 12]**

| | Quality evaluation | | | | | | | | | | |
|---|---|---|---|---|---|---|---|---|---|---|---|
| | Texture | Paper breakage | Cockle | Specific volume | Glossiness | Glossiness unevenness | Printing unevenness | Rigidity | Yellow change | Productivity | Overall evaluation |
| Example 9 | 5.6 | ○ | ○ | 1.26 | 60 | 4 | 3 | 65 | 5 | 4 | ⊚ |
| Example 10 | 5.6 | ○ | ○ | 1.25 | 62 | 4 | 4 | 66 | 5 | 4 | ⊚ |
| Example 11 | 5.5 | ○ | ○ | 1.23 | 62 | 5 | 5 | 65 | 5 | 4 | ⊚ |
| Example 12 | 5.6 | ○ | ○ | 1.20 | 62 | 5 | 5 | 66 | 5 | 4 | ⊚ |
| Example 13 | 5.6 | ○ | ○ | 1.19 | 60 | 4 | 4 | 65 | 5 | 4 | ⊚ |
| Example 14 | 5.5 | ○ | ○ | 1.16 | 62 | 4 | 4 | 65 | 5 | 4 | ⊚ |
| Example 15 | 5.6 | ○ | ○ | 1.15 | 63 | 4 | 5 | 65 | 5 | 4 | ⊚ |
| Example 16 | 5.6 | ○ | ○ | 1.13 | 62 | 5 | 5 | 66 | 5 | 4 | ⊚ |
| Example 17 | 5.6 | ○ | ○ | 1.09 | 62 | 5 | 5 | 65 | 5 | 4 | ⊚ |
| Example 18 | 5.6 | ○ | ○ | 1.07 | 62 | 5 | 5 | 65 | 5 | 4 | ⊚ |
| Example 19 | 5.6 | ○ | ○ | 1.04 | 61 | 5 | 4 | 64 | 5 | 4 | ⊚ |
| Example 20 | 5.5 | ○ | ○ | 1.02 | 61 | 4 | 4 | 63 | 5 | 4 | ⊚ |
| Example 21 | 5.5 | ○ | ○ | 1.02 | 61 | 4 | 4 | 63 | 4 | 4 | ○ |
| Example 22 | 5.4 | ○ | ○ | 1.02 | 61 | 4 | 4 | 62 | 4 | 4 | ○ |
| Example 23 | 5.4 | ○ | ○ | 1.01 | 60 | 4 | 3 | 62 | 4 | 4 | ○ |

**[Table 13]**

| | Wet paper forming step | | | Press part (1 P) | | Pre-dryer | Size press | After dryer | Pre-calender | Paper making speed |
|---|---|---|---|---|---|---|---|---|---|---|
| | Wire part mode | Suction mode | | | | | | | Soft calender | |
| | | 1 Stage | 2 Stage | Mode | Felt constitution | Mode | Mode | Mode | Mode | m/min |
| Example 24 | Gap former | Suction roll | Suction blade | Shoe press | Double felt | Single deck | Gate roll | Single deck | 1 Nip 1 stack | 1600 |
| Example 25 | Gap former | Suction roll | Suction blade | Shoe press | Double felt | Single deck | Gate roll | Single deck | 1 Nip 1 stack | 1600 |
| Example 26 | Gap former | Suction roll | Suction blade | Shoe press | Double felt | Single deck | Gate roll | Single deck | 1 Nip 1 stack | 1600 |
| Example 27 | Gap former | Suction roll | Suction blade | Shoe press | Double felt | Single deck | Gate roll | Single deck | 1 Nip 1 stack | 1600 |
| Example 28 | Gap former | Suction roll | Suction blade | Shoe press | Double felt | Single deck | Gate roll | Single deck | 1 Nip 1 stack | 1600 |
| Example 29 | Gap former | Suction roll | Suction blade | Shoe press | Double felt | Single deck | Gate roll | Single deck | 1 Nip 1 stack | 1600 |
| Example 30 | Gap former | Suction roll | Suction blade | Shoe press | Double felt | Single deck | Gate roll | Single deck | 1 Nip 1 stack | 1600 |
| Example 31 | Gap former | Suction roll | Suction blade | Shoe press | Double felt | Single deck | Gate roll | Single deck | 1 Nip 1 stack | 1600 |
| Example 32 | Gap former | Suction roll | Suction blade | Shoe press | Double felt | Single deck | Gate roll | Single deck | 1 Nip 1 stack | 1600 |
| Example 33 | Gap former | Suction roll | Suction blade | Shoe press | Double felt | Single deck | Gate roll | Single deck | 1 Nip 1 stack | 1600 |

**[Table 14]**

| | First coating apparatus | | | | Coating amount |
|---|---|---|---|---|---|
| | Coater mode | Hardness | Roll surface roughness | Material | Both faces |
| | | Hv | µm | | g/m² |
| Example 24 | Roll | 80 | 5 | Polyethylene blended urethane roll | 4 |
| Example 25 | Roll | 80 | 5 | Polyethylene blended urethane roll | 4 |
| Example 26 | Roll | 80 | 5 | Polyethylene blended urethane roll | 4 |
| Example 27 | Roll | 80 | 5 | Polyethylene blended urethane roll | 4 |
| Example 28 | Roll | 80 | 5 | Polyethylene blended urethane roll | 4 |
| Example 29 | Roll | 80 | 5 | Polyethylene blended urethane roll | 4 |
| Example 30 | Roll | 80 | 5 | Polyethylene blended urethane roll | 4 |
| Example 31 | Roll | 80 | 5 | Polyethylene blended urethane roll | 10 |
| Example 32 | Roll | 80 | 5 | Polyethylene blended urethane roll | 10 |
| Example 33 | Roll | 80 | 5 | Polyethylene blended urethane roll | 10 |

**[Table 15]**

| | Second coating apparatus (Front) | | | | | | |
|---|---|---|---|---|---|---|---|
| | Coating mode | Mode | Material | Thickness | Hardness | Bevel angle | Fountain angle |
| | | | | mm | Hv | | Degree |
| Example 24 | Jet fountain | Blade | Tungsten | 0.6 | 1400 | 40 | 50 |
| Example 25 | Jet fountain | Blade | Tungsten | 0.6 | 1400 | 40 | 50 |
| Example 26 | Jet fountain | Blade | Tungsten | 0.6 | 1400 | 40 | 50 |
| Example 27 | Jet fountain | Blade | Tungsten | 0.6 | 1400 | 40 | 50 |
| Example 28 | Jet fountain | Blade | Tungsten | 0.6 | 1400 | 40 | 50 |
| Example 29 | Jet fountain | Blade | Tungsten | 0.6 | 1400 | 40 | 50 |
| Example 30 | Jet fountain | Blade | Tungsten | 0.6 | 1400 | 40 | 50 |
| Example 31 | Jet fountain | Blade | Tungsten | 0.6 | 1400 | 40 | 50 |
| Example 32 | Jet fountain | Blade | Tungsten | 0.6 | 1400 | 40 | 50 |
| Example 33 | Jet fountain | Blade | Tungsten | 0.6 | 1400 | 40 | 50 |

**[Table 16]**

| | Second coating apparatus (Back) | | | | | | | Coating amount |
|---|---|---|---|---|---|---|---|---|
| | Coating mode | Mode | Material | Thickness | Hardness | Bevel angle | Fountain angle | Product coating amount |
| | | | | mm | Hv | | Degree | g/m² |
| Example 24 | Jet fountain | Blade | Tungsten | 0.6 | 1400 | 40 | 50 | 12 |
| Example 25 | Jet fountain | Blade | Tungsten | 0.6 | 1400 | 40 | 50 | 12 |
| Example 26 | Jet fountain | Blade | Tungsten | 0.6 | 1400 | 40 | 50 | 12 |
| Example 27 | Jet fountain | Blade | Tungsten | 0.6 | 1400 | 40 | 50 | 12 |
| Example 28 | Jet fountain | Blade | Tungsten | 0.6 | 1400 | 40 | 50 | 12 |
| Example 29 | Jet fountain | Blade | Tungsten | 0.6 | 1400 | 40 | 50 | 12 |
| Example 30 | Jet fountain | Blade | Tungsten | 0.6 | 1400 | 40 | 50 | 12 |
| Example 31 | Jet fountain | Blade | Tungsten | 0.6 | 1400 | 40 | 50 | 24 |
| Example 32 | Jet fountain | Blade | Tungsten | 0.6 | 1400 | 40 | 50 | 24 |
| Example 33 | Jet fountain | Blade | Tungsten | 0.6 | 1400 | 40 | 50 | 24 |

**[Table 17]**

| | Flattening treatment step | | | | Product grams per square meter | Raw material | | | Contaminant amount |
|---|---|---|---|---|---|---|---|---|---|
| | Stage number | Temperature | Surface roughness | Elastic roll hardness | | Waste paper | NBKP | LBKP | |
| | | °C | µm | Hv | g/m² | % | % | % | |
| Example 24 | 9 | 140 | 3 | 98 | 44 | 20 | 60 | 20 | 0.089 |
| Example 25 | 9 | 140 | 3 | 98 | 45 | 20 | 60 | 20 | 0.076 |
| Example 26 | 9 | 140 | 3 | 98 | 46 | 20 | 60 | 20 | 0.082 |
| Example 27 | 9 | 140 | 3 | 98 | 47 | 20 | 60 | 20 | 0.074 |
| Example 28 | 9 | 140 | 3 | 98 | 48 | 20 | 60 | 20 | 0.075 |
| Example 29 | 9 | 140 | 3 | 98 | 50 | 20 | 60 | 20 | 0.084 |
| Example 30 | 9 | 140 | 3 | 98 | 54 | 20 | 60 | 20 | 0.086 |
| Example 31 | 9 | 140 | 3 | 98 | 58 | 20 | 60 | 20 | 0.078 |
| Example 32 | 9 | 140 | 3 | 98 | 60 | 20 | 60 | 20 | 0.070 |
| Example 33 | 9 | 140 | 3 | 98 | 64 | 20 | 60 | 20 | 0.079 |

**[Table 18]**

| | Quality evaluation | | | | | | | | | | |
|---|---|---|---|---|---|---|---|---|---|---|---|
| | Texture | Paper breakage | Cockle | Specific volume | Glossiness | Glossiness unevenness | Printing unevenness | Rigidity | Yellow change | Productivity | Overall evaluation |
| Example 24 | 5.6 | ○ | ○ | 1.01 | 60 | 4 | 4 | 55 | 5 | 4 | ○ |
| Example 25 | 5.5 | ○ | ○ | 1.02 | 60 | 4 | 4 | 59 | 5 | 4 | ○ |
| Example 26 | 5.6 | ○ | ○ | 1.05 | 61 | 4 | 4 | 62 | 5 | 4 | ⊚ |
| Example 27 | 5.5 | ○ | ○ | 1.09 | 61 | 5 | 4 | 59 | 5 | 4 | ⊚ |
| Example 28 | 5.5 | ○ | ○ | 1.12 | 62 | 5 | 4 | 61 | 5 | 4 | ⊚ |
| Example 29 | 5.6 | ○ | ○ | 1.13 | 62 | 5 | 4 | 59 | 5 | 5 | ⊚ |
| Example 30 | 5.5 | ○ | ○ | 1.13 | 62 | 5 | 5 | 62 | 5 | 5 | ⊚ |
| Example 31 | 5.4 | ○ | ○ | 1.26 | 62 | 5 | 5 | 65 | 5 | 5 | ⊚ |
| Example 32 | 5.5 | ○ | ○ | 1.27 | 63 | 5 | 5 | 68 | 5 | 5 | ⊚ |
| Example 33 | 5.3 | ○ | ○ | 1.28 | 63 | 5 | 5 | 71 | 5 | 5 | ⊚ |

**[Table 19]**

| | Wet paper forming step | | | Press part (1 P) | | Pre-dryer | Size press | After dryer | Pre-calender | Paper making speed |
|---|---|---|---|---|---|---|---|---|---|---|
| | Wire part mode | Suction mode | | | | | | | Soft calender | |
| | | 1 Stage | 2 Stage | Mode | Felt constitution | Mode | Mode | Mode | Mode | m/min |
| Example 34 | Gap former | Suction roll | Suction blade | Shoe press | Double felt | Single deck | Gate roll | Single deck | 1 Nip 1 stack | 1000 |
| Example 35 | Gap former | Suction roll | Suction blade | Shoe press | Double felt | Single deck | Gate roll | Single deck | 1 Nip 1 stack | 1100 |
| Example 36 | Gap former | Suction roll | Suction blade | Shoe press | Double felt | Single deck | Gate roll | Single deck | 1 Nip 1 stack | 1200 |
| Example 37 | Gap former | Suction roll | Suction blade | Shoe press | Double felt | Single deck | Gate roll | Single deck | 1 Nip 1 stack | 1300 |
| Example 38 | Gap former | Suction roll | Suction blade | Shoe press | Double felt | Single deck | Gate roll | Single deck | 1 Nip 1 stack | 1400 |
| Example 39 | Gap former | Suction roll | Suction blade | Shoe press | Double felt | Single deck | Gate roll | Single deck | 1 Nip 1 stack | 1500 |
| Example 40 | Gap former | Suction roll | Suction blade | Shoe press | Double felt | Single deck | Gate roll | Single deck | 1 Nip 1 stack | 1600 |
| Example 41 | Gap former | Suction roll | Suction blade | Shoe press | Double felt | Single deck | Gate roll | Single deck | 1 Nip 1 stack | 1700 |
| Example 42 | Gap former | Suction roll | Suction blade | Shoe press | Double felt | Single deck | Gate roll | Single deck | 1 Nip 1 stack | 1800 |

**[Table 20]**

| | First coating apparatus | | | | Coating amount |
|---|---|---|---|---|---|
| | Coater mode | Hardness | Roll surface roughness | Material | Both faces |
| | | Hv | µm | | g/m² |
| Example 34 | Roll | 80 | 5 | Polyethylene blended urethane roll | 4 |
| Example 35 | Roll | 80 | 5 | Polyethylene blended urethane roll | 4 |
| Example 36 | Roll | 80 | 5 | Polyethylene blended urethane roll | 4 |
| Example 37 | Roll | 80 | 5 | Polyethylene blended urethane roll | 4 |
| Example 38 | Roll | 80 | 5 | Polyethylene blended urethane roll | 4 |
| Example 39 | Roll | 80 | 5 | Polyethylene blended urethane roll | 4 |
| Example 40 | Roll | 80 | 5 | Polyethylene blended urethane roll | 4 |
| Example 41 | Roll | 80 | 5 | Polyethylene blended urethane roll | 4 |
| Example 42 | Roll | 80 | 5 | Polyethylene blended urethane roll | 4 |

**[Table 21]**

| | Second coating apparatus (Front) | | | | | | |
|---|---|---|---|---|---|---|---|
| | Coating mode | Mode | Material | Thickness | Hardness | Bevel angle | Fountain angle |
| | | | | mm | Hv | | Degree |
| Example 34 | Jet fountain | Blade | Tungsten | 0.6 | 1400 | 40 | 50 |
| Example 35 | Jet fountain | Blade | Tungsten | 0.6 | 1400 | 40 | 50 |
| Example 36 | Jet fountain | Blade | Tungsten | 0.6 | 1400 | 40 | 50 |
| Example 37 | Jet fountain | Blade | Tungsten | 0.6 | 1400 | 40 | 50 |
| Example 38 | Jet fountain | Blade | Tungsten | 0.6 | 1400 | 40 | 50 |
| Example 39 | Jet fountain | Blade | Tungsten | 0.6 | 1400 | 40 | 50 |
| Example 40 | Jet fountain | Blade | Tungsten | 0.6 | 1400 | 40 | 50 |
| Example 41 | Jet fountain | Blade | Tungsten | 0.6 | 1400 | 40 | 50 |
| Example 42 | Jet fountain | Blade | Tungsten | 0.6 | 1400 | 40 | 50 |

**[Table 22]**

| | Second coating apparatus (Back) | | | | | | | Coating amount |
|---|---|---|---|---|---|---|---|---|
| | Coating mode | Mode | Material | Thickness | Hardness | Bevel angle | Fountain angle | Product coating amount |
| | | | | mm | Hv | | Degree | g/m² |
| Example 34 | Jet fountain | Blade | Tungsten | 0.6 | 1400 | 40 | 50 | 12 |
| Example 35 | Jet fountain | Blade | Tungsten | 0.6 | 1400 | 40 | 50 | 12 |
| Example 36 | Jet fountain | Blade | Tungsten | 0.6 | 1400 | 40 | 50 | 12 |
| Example 37 | Jet fountain | Blade | Tungsten | 0.6 | 1400 | 40 | 50 | 12 |
| Example 38 | Jet fountain | Blade | Tungsten | 0.6 | 1400 | 40 | 50 | 12 |
| Example 39 | Jet fountain | Blade | Tungsten | 0.6 | 1400 | 40 | 50 | 12 |
| Example 40 | Jet fountain | Blade | Tungsten | 0.6 | 1400 | 40 | 50 | 12 |
| Example 41 | Jet fountain | Blade | Tungsten | 0.6 | 1400 | 40 | 50 | 12 |
| Example 42 | Jet fountain | Blade | Tungsten | 0.6 | 1400 | 40 | 50 | 12 |

**[Table 23]**

| | Flattening treatment step | | | | Product grams per square meter | Raw material | | | Contaminant amount |
|---|---|---|---|---|---|---|---|---|---|
| | Stage number | Temperature | Surface roughness | Elastic roll hardness | | Waste paper | NBKP | LBKP | |
| | | °C | µm | Hv | g/m² | % | % | % | |
| Example 34 | 9 | 140 | 3 | 98 | 54 | 20 | 60 | 20 | 0.071 |
| Example 35 | 9 | 140 | 3 | 98 | 54 | 20 | 60 | 20 | 0.087 |
| Example 36 | 9 | 140 | 3 | 98 | 54 | 20 | 60 | 20 | 0.072 |
| Example 37 | 9 | 140 | 3 | 98 | 54 | 20 | 60 | 20 | 0.078 |
| Example 38 | 9 | 140 | 3 | 98 | 54 | 20 | 60 | 20 | 0.087 |
| Example 39 | 9 | 140 | 3 | 98 | 54 | 20 | 60 | 20 | 0.071 |
| Example 40 | 9 | 140 | 3 | 98 | 54 | 20 | 60 | 20 | 0.075 |
| Example 41 | 9 | 140 | 3 | 98 | 54 | 20 | 60 | 20 | 0.088 |
| Example 42 | 9 | 140 | 3 | 98 | 54 | 20 | 60 | 20 | 0.077 |

**[Table 24]**

| | Quality evaluation | | | | | | | | | | |
|---|---|---|---|---|---|---|---|---|---|---|---|
| | Texture | Paper breakage | Cockle | Specific volume | Glossiness | Glossiness unevenness | Printing unevenness | Rigidity | Yellow change | Productivity | Overall evaluation |
| Example 34 | 5.5 | ○ | ○ | 1.11 | 64 | 5 | 5 | 55 | 5 | 3 | ○ |
| Example 35 | 5.4 | ○ | ○ | 1.14 | 63 | 5 | 5 | 56 | 5 | 3 | ○ |
| Example 36 | 5.4 | ○ | ○ | 1.15 | 63 | 5 | 5 | 60 | 5 | 4 | ⊚ |
| Example 37 | 5.5 | ○ | ○ | 1.16 | 62 | 5 | 5 | 63 | 5 | 4 | ⊚ |
| Example 38 | 5.5 | ○ | ○ | 1.17 | 62 | 5 | 5 | 63 | 5 | 5 | ⊚ |
| Example 39 | 5.5 | ○ | ○ | 1.19 | 62 | 5 | 5 | 64 | 5 | 5 | ⊚ |
| Example 40 | 5.4 | ○ | ○ | 1.22 | 61 | 5 | 5 | 65 | 5 | 5 | ⊚ |
| Example 41 | 5.4 | ○ | ○ | 1.25 | 61 | 5 | 5 | 66 | 5 | 5 | ⊚ |
| Example 42 | 5.5 | ○ | ○ | 1.28 | 60 | 4 | 4 | 68 | 5 | 5 | ○ |

**[Table 25]**

| | Wet paper forming step | | | Press part (1 P) | | Pre-dryer | Size press | After dryer | Pre-calender | Paper making speed |
|---|---|---|---|---|---|---|---|---|---|---|
| | Wire part mode | Suction mode | | | | | | | Soft calender | |
| | | 1 Stage | 2 Stage | Mode | Felt constitution | Mode | Mode | Mode | Mode | m/min |
| Example 43 | Gap former | Suction roll | Suction blade | Shoe press | Double felt | Single deck | Gate roll | Single deck | 1 Nip 1 stack | 1600 |
| Example 44 | Gap former | Suction roll | Suction blade | Shoe press | Double felt | Single deck | Gate roll | Single deck | 1 Nip 1 stack | 1600 |
| Example 45 | Gap former | Suction roll | Suction blade | Shoe press | Double felt | Single deck | Gate roll | Single deck | 1 Nip 1 stack | 1600 |
| Example 46 | Gap former | Suction roll | Suction blade | Shoe press | Double felt | Single deck | Gate roll | Single deck | 1 Nip 1 stack | 1600 |
| Example 47 | Gap former | Suction roll | Suction blade | Shoe press | Double felt | Single deck | Gate roll | Single deck | 1 Nip 1 stack | 1600 |
| Example 48 | Gap former | Suction roll | Suction blade | Shoe press | Double felt | Single deck | Gate roll | Single deck | 1 Nip 1 stack | 1600 |
| Example 49 | Gap former | Suction roll | Suction blade | Shoe press | Double felt | Single deck | Gate roll | Single deck | 1 Nip 1 stack | 1600 |
| Example 50 | Gap former | Suction roll | Suction blade | Shoe press | Double felt | Single deck | Gate roll | Single deck | 1 Nip 1 stack | 1800 |
| Example 51 | Gap former | Suction roll | Suction blade | Shoe press | Double felt | Single deck | Gate roll | Single deck | 1 Nip 1 stack | 1300 |
| Example 52 | Gap former | Suction roll | Suction blade | Shoe press | Double felt | Single deck | Gate roll | Single deck | 1 Nip 1 stack | 1600 |
| Example 53 | Gap former | Suction roll | Suction blade | Shoe press | Double felt | Single deck | Gate roll | Single deck | 1 Nip 1 stack | 1600 |
| Example 54 | Gap former | Suction roll | Suction blade | Shoe press | Double felt | Single deck | Gate roll | Single deck | 1 Nip 1 stack | 1600 |
| Example 55 | Gap former | Suction roll | Suction blade | Shoe press | Double felt | Single deck | Gate roll | Single deck | 1 Nip 1 stack | 1600 |
| Example 56 | Gap former | Suction roll | Suction blade | Shoe press | Double felt | Single deck | Gate roll | Single deck | 1 Nip 1 stack | 1600 |
| Example 57 | Gap former | Suction roll | Suction blade | Shoe press | Double felt | Single deck | Gate roll | Single deck | 1 Nip 1 stack | 1600 |
| Example 58 | Gap former | Suction roll | Suction blade | Shoe press | Double felt | Single deck | Gate roll | Single deck | 1 Nip 1 stack | 1600 |
| Example 59 | Gap former | Suction roll | Suction blade | Shoe press | Double felt | Single deck | Gate roll | Single deck | 1 Nip 1 stack | 1600 |
| Example 60 | Gap former | Suction roll | Suction blade | Shoe press | Double felt | Single deck | Gate roll | Single deck | 1 Nip 1 stack | 1600 |
| Example 61 | Gap former | Suction roll | Suction blade | Shoe press | Double felt | Single deck | Gate roll | Single deck | 1 Nip 1 stack | 1600 |
| Example 62 | Gap former | Suction roll | Suction blade | Shoe press | Double felt | Single deck | Gate roll | Single deck | 1 Nip 1 stack | 1600 |
| Example 63 | Gap former | Suction roll | Suction blade | Shoe press | Double felt | Single deck | Gate roll | Single deck | 1 Nip 1 stack | 1800 |
| Example 64 | Gap former | Suction roll | Suction blade | Shoe press | Double felt | Single deck | Gate roll | Single deck | 1 Nip 1 stack | 1300 |
| Example 65 | Gap former | Suction roll | Suction blade | Shoe press | Double felt | Single deck | Gate roll | Single deck | 1 Nip 1 stack | 1600 |
| Example 66 | Gap former | Suction roll | Suction blade | Shoe press | Double felt | Single deck | Gate roll | Single deck | 1 Nip 1 stack | 1600 |
| Example 67 | Gap former | Suction roll | Suction blade | Shoe press | Double felt | Single deck | Gate roll | Single deck | 1 Nip 1 stack | 1600 |
| Example 68 | Gap former | Suction roll | Suction blade | Shoe press | Double felt | Single deck | Gate roll | Single deck | 1 Nip 1 stack | 1600 |
| Example 69 | Gap former | Suction roll | Suction blade | Shoe press | Double felt | Single deck | Gate roll | Single deck | 1 Nip 1 stack | 1600 |

**[Table 26]**

| | First coating apparatus | | | | Coating amount |
|---|---|---|---|---|---|
| | Coater mode | Hardness | Roll surface roughness | Material | Both faces |
| | | Hv | µm | | g/m² |
| Example 43 | Roll | 80 | 5 | Polyethylene blended urethane roll | 4 |
| Example 44 | Roll | 80 | 5 | Polyethylene blended urethane roll | 8 |
| Example 45 | Roll | 80 | 5 | Polyethylene blended urethane roll | 10 |
| Example 46 | Roll | 80 | 5 | Polyethylene blended urethane roll | 12 |
| Example 47 | Roll | 80 | 5 | Polyethylene blended urethane roll | 14 |
| Example 48 | Roll | 80 | 5 | Polyethylene blended urethane roll | 18 |
| Example 49 | Roll | 80 | 5 | Polyethylene blended urethane roll | 20 |
| Example 50 | Roll | 80 | 5 | Polyethylene blended urethane roll | 10 |
| Example 51 | Roll | 80 | 5 | Polyethylene blended urethane roll | 10 |
| Example 52 | Roll | 80 | 5 | Polyethylene blended urethane roll | 10 |
| Example 53 | Roll | 80 | 5 | Polyethylene blended urethane roll | 10 |
| Example 54 | Roll | 80 | 5 | Polyethylene blended urethane roll | 10 |
| Example 55 | Roll | 80 | 5 | Polyethylene blended urethane roll | 10 |
| Example 56 | Roll | 80 | 5 | Polyethylene blended urethane roll | 10 |
| Example 57 | - | - | - | - | - |
| Example 58 | - | - | - | - | - |
| Example 59 | - | - | - | - | - |
| Example 60 | - | - | - | - | - |
| Example 61 | - | - | - | - | - |
| Example 62 | - | - | - | - | - |
| Example 63 | - | - | - | - | - |
| Example 64 | - | - | - | - | - |
| Example 65 | - | - | - | - | - |
| Example 66 | - | - | - | - | - |
| Example 67 | - | - | - | - | - |
| Example 68 | - | - | - | - | - |
| Example 69 | - | - | - | - | - |

**[Table 27]**

| | Second coating apparatus | | | | | | |
|---|---|---|---|---|---|---|---|
| | Coating mode | Mode | Material | Thickness | Hardness | Bevel angle | Fountain angle |
| | | | | mm | Hv | | Degree |
| Example 43 | - | - | - | - | - | - | - |
| Example 44 | - | - | - | - | - | - | - |
| Example 45 | - | - | - | - | - | - | - |
| Example 46 | - | - | - | - | - | - | - |
| Example 47 | - | - | - | - | - | - | - |
| Example 48 | - | - | - | - | - | - | - |
| Example 49 | - | - | - | - | - | - | - |
| Example 50 | - | - | - | - | - | - | - |
| Example 51 | - | - | - | - | - | - | - |
| Example 52 | - | - | - | - | - | - | - |
| Example 53 | - | - | - | - | - | - | - |
| Example 54 | - | - | - | - | - | - | - |
| Example 55 | - | - | - | - | - | - | - |
| Example 56 | - | - | - | - | - | - | - |
| Example 57 | Jet fountain | Blade | Tungsten | 0.6 | 1400 | 40 | 50 |
| Example 58 | Jet fountain | Blade | Tungsten | 0.6 | 1400 | 40 | 50 |
| Example 59 | Jet fountain | Blade | Tungsten | 0.6 | 1400 | 40 | 50 |
| Example 60 | Jet fountain | Blade | Tungsten | 0.6 | 1400 | 40 | 50 |
| Example 61 | Jet fountain | Blade | Tungsten | 0.6 | 1400 | 40 | 50 |
| Example 62 | Jet fountain | Blade | Tungsten | 0.6 | 1400 | 40 | 50 |
| Example 63 | Jet fountain | Blade | Tungsten | 0.6 | 1400 | 40 | 50 |
| Example 64 | Jet fountain | Blade | Tungsten | 0.6 | 1400 | 40 | 50 |
| Example 65 | Jet fountain | Blade | Tungsten | 0.6 | 1400 | 40 | 50 |
| Example 66 | Jet fountain | Blade | Tungsten | 0.6 | 1400 | 40 | 50 |
| Example 67 | Jet fountain | Blade | Tungsten | 0.6 | 1400 | 40 | 50 |
| Example 68 | Jet fountain | Blade | Tungsten | 0.6 | 1400 | 40 | 50 |
| Example 69 | Jet fountain | Blade | Tungsten | 0.6 | 1400 | 40 | 50 |

**[Table 28]**

| | Second coating apparatus (Back) | | | | | | | Coating amount |
|---|---|---|---|---|---|---|---|---|
| | Coating mode | Mode | Material | Thickness | Hardness | Bevel angle | Fountain angle | Product coating amount |
| | | | | mm | Hv | | Degree | g/m² |
| Example 43 | - | - | - | - | - | - | - | 4 |
| Example 44 | - | - | - | - | - | - | - | 8 |
| Example 45 | - | - | - | - | - | - | - | 10 |
| Example 46 | - | - | - | - | - | - | - | 12 |
| Example 47 | - | - | - | - | - | - | - | 14 |
| Example 48 | - | - | - | - | - | - | - | 18 |
| Example 49 | - | - | - | - | - | - | - | 20 |
| Example 50 | - | - | - | - | - | - | - | 10 |
| Example 51 | - | - | - | - | - | - | - | 10 |
| Example 52 | - | - | - | - | - | - | - | 10 |
| Example 53 | - | - | - | - | - | - | - | 10 |
| Example 54 | - | - | - | - | - | - | - | 10 |
| Example 55 | - | - | - | - | - | - | - | 10 |
| Example 56 | - | - | - | - | - | - | - | 10 |
| Example 57 | Jet fountain | Blade | Tungsten | 0.6 | 1400 | 40 | 50 | 12 |
| Example 58 | Jet fountain | Blade | Tungsten | 0.6 | 1400 | 40 | 50 | 14 |
| Example 59 | Jet fountain | Blade | Tungsten | 0.6 | 1400 | 40 | 50 | 15 |
| Example 60 | Jet fountain | Blade | Tungsten | 0.6 | 1400 | 40 | 50 | 20 |
| Example 61 | Jet fountain | Blade | Tungsten | 0.6 | 1400 | 40 | 50 | 25 |
| Example 62 | Jet fountain | Blade | Tungsten | 0.6 | 1400 | 40 | 50 | 30 |
| Example 63 | Jet fountain | Blade | Tungsten | 0.6 | 1400 | 40 | 50 | 12 |
| Example 64 | Jet fountain | Blade | Tungsten | 0.6 | 1400 | 40 | 50 | 12 |
| Example 65 | Jet fountain | Blade | Tungsten | 0.6 | 1400 | 40 | 50 | 12 |
| Example 66 | Jet fountain | Blade | Tungsten | 0.6 | 1400 | 40 | 50 | 12 |
| Example 67 | Jet fountain | Blade | Tungsten | 0.6 | 1400 | 40 | 50 | 12 |
| Example 68 | Jet fountain | Blade | Tungsten | 0.6 | 1400 | 40 | 50 | 12 |
| Example 69 | Jet fountain | Blade | Tungsten | 0.6 | 1400 | 40 | 50 | 12 |

**[Table 29]**

| | Flattening treatment step | | | | Product grams per square meter | Raw material | | | Contaminant amount |
|---|---|---|---|---|---|---|---|---|---|
| | Stage number | Temperature | Surface roughness | Elastic roll hardness | | Waste paper | NBKP | LBKP | |
| | | °C | µm | Hv | g/m² | % | % | % | |
| Example 43 | 9 | 140 | 3 | 98 | 30 | 20 | 60 | 20 | 0.086 |
| Example 44 | 9 | 140 | 3 | 98 | 38 | 20 | 60 | 20 | 0.082 |
| Example 45 | 9 | 140 | 3 | 98 | 40.2 | 20 | 60 | 20 | 0.082 |
| Example 46 | 9 | 140 | 3 | 98 | 42 | 20 | 60 | 20 | 0.089 |
| Example 47 | 9 | 140 | 3 | 98 | 44 | 20 | 60 | 20 | 0.077 |
| Example 48 | 9 | 140 | 3 | 98 | 48 | 20 | 60 | 20 | 0.084 |
| Example 49 | 9 | 140 | 3 | 98 | 54.2 | 20 | 60 | 20 | 0.075 |
| Example 50 | 9 | 140 | 3 | 98 | 54.2 | 20 | 60 | 20 | 0.082 |
| Example 51 | 9 | 140 | 3 | 98 | 54.2 | 20 | 60 | 20 | 0.082 |
| Example 52 | 9 | 140 | 3 | 98 | 35 | 20 | 60 | 20 | 0.076 |
| Example 53 | 9 | 140 | 3 | 98 | 64 | 20 | 60 | 20 | 0.087 |
| Example 54 | 9 | 140 | 3 | 98 | 54.2 | 40 | 40 | 20 | 0.083 |
| Example 55 | 9 | 140 | 3 | 98 | 54.2 | 50 | 30 | 20 | 0.081 |
| Example 56 | 9 | 140 | 3 | 98 | 54.2 | 100 | - | - | 0.074 |
| Example 57 | 9 | 140 | 3 | 98 | 54.2 | 20 | 50 | 30 | 0.071 |
| Example 58 | 9 | 140 | 3 | 98 | 54.2 | 20 | 50 | 30 | 0.081 |
| Example 59 | 9 | 140 | 3 | 98 | 54.2 | 20 | 50 | 30 | 0.072 |
| Example 60 | 9 | 140 | 3 | 98 | 54.2 | 20 | 50 | 30 | 0.086 |
| Example 61 | 9 | 140 | 3 | 98 | 54.2 | 20 | 50 | 30 | 0.070 |
| Example 62 | 9 | 140 | 3 | 98 | 54.2 | 20 | 50 | 30 | 0.088 |
| Example 63 | 9 | 140 | 3 | 98 | 54.2 | 20 | 60 | 20 | 0.082 |
| Example 64 | 9 | 140 | 3 | 98 | 54.2 | 20 | 60 | 20 | 0.082 |
| Example 65 | 9 | 140 | 3 | 98 | 40 | 20 | 60 | 20 | 0.076 |
| Example 66 | 9 | 140 | 3 | 98 | 64 | 20 | 60 | 20 | 0.087 |
| Example 67 | 9 | 140 | 3 | 98 | 54.2 | 40 | 40 | 20 | 0.082 |
| Example 68 | 9 | 140 | 3 | 98 | 54.2 | 50 | 30 | 20 | 0.079 |
| Example 69 | 9 | 140 | 3 | 98 | 54.2 | 100 | - | - | 0.073 |

**[Table 30]**

| | Quality evaluation | | | | | | | | | | |
|---|---|---|---|---|---|---|---|---|---|---|---|
| | Texture | Paper breakage | Cockle | Specific volume | Glossiness | Glossiness unevenness | Printing unevenness | Rigidity | Yellow change | Productivity | Overall evaluation |
| Example 43 | 5.6 | ○ | ○ | 1.26 | 57 | 4 | 3 | 66 | 5 | 4 | ○ |
| Example 44 | 5.6 | ○ | ○ | 1.24 | 56 | 4 | 4 | 64 | 4 | 4 | ○ |
| Example 45 | 5.5 | ○ | ○ | 1.23 | 56 | 4 | 4 | 63 | 4 | 4 | ○ |
| Example 46 | 5.6 | ○ | ○ | 1.20 | 56 | 4 | 4 | 65 | 5 | 4 | ○ |
| Example 47 | 5.5 | ○ | ○ | 1.26 | 56 | 4 | 4 | 64 | 5 | 4 | ○ |
| Example 48 | 5.5 | ○ | ○ | .24 | 57 | 3 | 4 | 64 | 5 | 4 | ○ |
| Example 49 | 5.6 | ○ | ○ | 1.23 | 57 | 3 | 3 | 63 | 4 | 4 | ○ |
| Example 50 | 5.5 | ○ | ○ | 1.23 | 56 | 4 | 4 | 63 | 4 | 4 | ○ |
| Example 51 | 5.5 | ○ | ○ | 1.23 | 56 | 4 | 4 | 63 | 4 | 4 | ○ |
| Example 52 | 5.5 | ○ | ○ | 1.23 | 55 | 4 | 4 | 64 | 4 | 4 | ○ |
| Example 53 | 5.5 | ○ | ○ | 1.23 | 56 | 4 | 4 | 63 | 4 | 4 | ○ |
| Example 54 | 5.6 | ○ | ○ | 1.23 | 56 | 4 | 4 | 64 | 4 | 4 | ○ |
| Example 55 | 5.5 | ○ | ○ | 1.20 | 56 | 4 | 4 | 63 | 4 | 4 | ○ |
| Example 56 | 5.5 | ○ | ○ | 1.23 | 56 | 4 | 4 | 63 | 4 | 4 | ○ |
| Example 57 | 5.6 | ○ | ○ | 1.19 | 61 | 4 | 4 | 65 | 5 | 4 | ○ |
| Example 58 | 5.6 | ○ | ○ | 1.24 | 62 | 5 | 5 | 64 | 5 | 4 | ○ |
| Example 59 | 5.6 | ○ | ○ | 1.22 | 62 | 5 | 5 | 64 | 5 | 4 | ○ |
| Example 60 | 5.6 | ○ | ○ | 1.21 | 62 | 5 | 5 | 63 | 5 | 4 | ○ |
| Example 61 | 5.6 | ○ | ○ | 1.18 | 63 | 5 | 5 | 63 | 5 | 4 | ○ |
| Example 62 | 5.6 | ○ | ○ | 1.16 | 63 | 5 | 5 | 62 | 5 | 4 | ○ |
| Example 63 | 5.5 | ○ | ○ | 1.23 | 60 | 4 | 4 | 63 | 4 | 4 | ○ |
| Example 64 | 5.5 | ○ | ○ | 1.23 | 61 | 4 | 4 | 63 | 4 | 4 | ○ |
| Example 65 | 5.5 | ○ | ○ | 1.20 | 62 | 4 | 4 | 63 | 4 | 4 | ○ |
| Example 66 | 5.5 | ○ | ○ | 1.23 | 62 | 4 | 4 | 64 | 4 | 4 | ○ |
| Example 67 | 5.6 | ○ | ○ | 1.23 | 61 | 4 | 4 | 64 | 4 | 4 | ○ |
| Example 68 | 5.5 | ○ | ○ | 1.23 | 62 | 4 | 4 | 63 | 4 | 4 | ○ |
| Example 69 | 5.5 | ○ | ○ | 1.20 | 61 | 4 | 4 | 63 | 4 | 4 | ○ |

**[Table 31]**

| | Wet paper forming step | | | Press part (1 P) | | Pre-dryer | Size press | After dryer | Pre-calender | Paper making speed |
|---|---|---|---|---|---|---|---|---|---|---|
| | Wire part mode | Suction mode | | | | | | | Soft calender | |
| | | 1 Stage | 2 Stage | Mode | Felt constitution | Mode | Mode | Mode | Mode | m/min |
| Comparative Example 8 | Gap former | Suction roll | Suction blade | Shoe press | Double felt | Single deck | Gate roll | Single deck | - | 800 |
| Comparative Example 9 | Gap former | Suction roll | Suction blade | Shoe press | Double felt | Single deck | Gate roll | Single deck | - | 1200 |
| Comparative Example 10 | Gap former | Suction roll | Suction blade | Shoe press | Double felt | Single deck | - | Single deck | 1 Nip 1 stack | 1600 |
| Comparative Example 11 | Gap former | Suction roll | Suction blade | Shoe press | Double felt | Single deck | - | Single deck | 1 Nip 1 stack | 1800 |
| Comparative Example 12 | Gap former | Suction roll | Suction blade | Shoe press | Double felt | Single deck | - | Single deck | 1 Nip 1 stack | 1600 |
| Comparative Example 13 | Gap former | Suction roll | Suction blade | Shoe press | Double felt | Single deck | - | Single deck | 1 Nip 1 stack | 1600 |
| Comparative Example 14 | Gap former | Suction roll | Suction blade | Shoe press | Double felt | Single deck | Gate roll | Single deck | 1 Nip 1 stack | 1600 |
| Comparative Example 15 | Gap former | Suction roll | Suction blade | Shoe press | Double felt | Single deck | Gate roll | Single deck | - | 800 |
| Comparative Example 16 | Gap former | Suction roll | Suction blade | Shoe press | Double felt | Single deck | Gate roll | Single deck | - | 1200 |
| Comparative Example 17 | Gap former | Suction roll | Suction blade | Shoe press | Double felt | Single deck | - | Single deck | 1 Nip 1 stack | 1600 |
| Comparative Example 18 | Gap former | Suction roll | Suction blade | Shoe press | Double felt | Single deck | - | Single deck | 1 Nip 1 stack | 1800 |
| Comparative Example 19 | Gap former | Suction roll | Suction blade | Shoe press | Double felt | Single deck | - | Single deck | 1 Nip 1 stack | 1600 |
| Comparative Example 20 | Gap former | Suction roll | Suction blade | Shoe press | Double felt | Single deck | - | Single deck | 1 Nip 1 stack | 1600 |
| Comparative Example 21 | Gap former | Suction roll | Suction blade | Shoe press | Double felt | Single deck | Gate roll | Single deck | 1 Nip 1 stack | 1600 |
| Comparative Example 22 | Gap former | Suction roll | Suction blade | Shoe press | Double felt | Single deck | - | Single deck | - | 1600 |
| Comparative Example 23 | Gap former | Suction roll | Suction blade | Shoe press | Double felt | Single deck | - | Single deck | - | 1600 |
| Comparative Example 24 | Gap former | Suction roll | Suction blade | Shoe press | Double felt | Single deck | - | Single deck | - | 1600 |
| Comparative Example 25 | Gap former | Suction roll | Suction blade | Shoe press | Double felt | Single deck | - | Single deck | - | 1600 |
| Comparative Example 26 | Gap former | Suction roll | Suction blade | Shoe press | Double felt | Single deck | - | Single deck | - | 1600 |
| Comparative Example 27 | Gap former | Suction roll | Suction blade | Shoe press | Double felt | Single deck | Gate roll | Single deck | 1 Nip 1 stack | 1600 |

**[Table 32]**

| | First coating apparatus | | | | Coating amount |
|---|---|---|---|---|---|
| | Coater mode | Hardness | Roll surface roughness | Material | Both faces |
| | | Hv | µm | | g/m² |
| Comparative Example 8 | - | - | - | - | - |
| Comparative Example 9 | - | - | - | - | - |
| Comparative Example 10 | - | - | - | - | - |
| Comparative Example 11 | - | - | - | - | - |
| Comparative Example 12 | - | - | - | - | - |
| Comparative Example 13 | - | - | - | - | - |
| Comparative Example 14 | - | - | - | - | - |
| Comparative Example 15 | Roll | 80 | 5 | Polyethylene blended urethane roll | 10 |
| Comparative Example 16 | Roll | 80 | 5 | Polyethylene blended urethane roll | 10 |
| Comparative Example 17 | Roll | 80 | 5 | Polyethylene blended urethane roll | 10 |
| Comparative Example 18 | Roll | 80 | 5 | Polyethylene blended urethane roll | 10 |
| Comparative Example 19 | Roll | 80 | 5 | Polyethylene blended urethane roll | 22 |
| Comparative Example 20 | Roll | 80 | 5 | Polyethylene blended urethane roll | 24 |
| Comparative Example 21 | Roll | 80 | 5 | Polyethylene blended urethane roll | 10 |
| Comparative Example 22 | Roll | 80 | 5 | Polyethylene blended urethane roll | 10 |
| Comparative Example 23 | Roll | 80 | 5 | Polyethylene blended urethane roll | 10 |
| Comparative Example 24 | Roll | 80 | 5 | Polyethylene blended urethane roll | 10 |
| Comparative Example 25 | Roll | 80 | 5 | Polyethylene blended urethane roll | 10 |
| Comparative Example 26 | Roll | 80 | 5 | Polyethylene blended urethane roll | 10 |
| Comparative Example 27 | Roll | 80 | 5 | Polyethylene blended urethane roll | 10 |

**[Table 33]**

| | Second coating apparatus | | | | | | |
|---|---|---|---|---|---|---|---|
| | Coating mode | Mode | Material | Thickness | Hardness | Bevel angle | Fountain angle |
| | | | | mm | Hv | | Degree |
| Comparative Example 8 | Jet fountain | Blade | Tungsten | 0.6 | 1400 | 40 | 50 |
| Comparative Example 9 | Jet fountain | Blade | Tungsten | 0.6 | 1400 | 40 | 50 |
| Comparative Example 10 | Jet fountain | Blade | Tungsten | 0.6 | 1400 | 40 | 50 |
| Comparative Example 11 | Jet fountain | Blade | Tungsten | 0.6 | 1400 | 40 | 50 |
| Comparative Example 12 | Jet fountain | Blade | Tungsten | 0.6 | 1400 | 40 | 50 |
| Comparative Example 13 | Jet fountain | Blade | Tungsten | 0.6 | 1400 | 40 | 50 |
| Comparative Example 14 | Jet fountain | Blade | Tungsten | 0.6 | 1400 | 40 | 50 |
| Comparative Example 15 | - | - | - | - | - | - | - |
| Comparative Example 16 | - | - | - | - | - | - | - |
| Comparative Example 17 | - | - | - | - | - | - | - |
| Comparative Example 18 | - | - | - | - | - | - | - |
| Comparative Example 19 | - | - | - | - | - | - | - |
| Comparative Example 20 | - | - | - | - | - | - | - |
| Comparative Example 21 | - | - | - | - | - | - | - |
| Comparative Example 22 | Jet fountain | Blade | Tungsten | 0.6 | 1400 | 40 | 50 |
| Comparative Example 23 | Jet fountain | Blade | Tungsten | 0.6 | 1400 | 40 | 50 |
| Comparative Example 24 | Jet fountain | Blade | Tungsten | 0.6 | 1400 | 40 | 50 |
| Comparative Example 25 | Jet fountain | Blade | Tungsten | 0.6 | 1400 | 40 | 50 |
| Comparative Example 26 | Jet fountain | Blade | Tungsten | 0.6 | 1400 | 40 | 50 |
| Comparative Example 27 | Jet fountain | Blade | Tungsten | 0.6 | 1400 | 40 | 50 |

**[Table 34]**

| | Second coating apparatus (Back) | | | | | | | Coating amount |
|---|---|---|---|---|---|---|---|---|
| | Coating mode | Mode | Material | Thickness | Hardness | Bevel angle | Fountain angle | Product coating amount |
| | | | | mm | Hv | | Degree | g/m² |
| Comparative Example 8 | Jet fountain | Blade | Tungsten | 0.6 | 1400 | 40 | 50 | 12 |
| Comparative Example 9 | Jet fountain | Blade | Tungsten | 0.6 | 1400 | 40 | 50 | 12 |
| Comparative Example 10 | Jet fountain | Blade | Tungsten | 0.6 | 1400 | 40 | 50 | 12 |
| Comparative Example 11 | Jet fountain | Blade | Tungsten | 0.6 | 1400 | 40 | 50 | 12 |
| Comparative Example 12 | Jet fountain | Blade | Tungsten | 0.6 | 1400 | 40 | 50 | 22 |
| Comparative Example 13 | Jet fountain | Blade | Tungsten | 0.6 | 1400 | 40 | 50 | 24 |
| Comparative Example 14 | Jet fountain | Blade | Tungsten | 0.6 | 1400 | 40 | 50 | 12 |
| Comparative Example 15 | - | - | - | - | - | - | - | 10 |
| Comparative Example 16 | - | - | - | - | - | - | - | 10 |
| Comparative Example 17 | - | - | - | - | - | - | - | 10 |
| Comparative Example 18 | - | - | - | - | - | - | - | 10 |
| Comparative Example 19 | - | - | - | - | - | - | - | 22 |
| Comparative Example 20 | - | - | - | - | - | - | - | 24 |
| Comparative Example 21 | - | - | - | - | - | - | - | 10 |
| Comparative Example 22 | Jet fountain | Blade | Tungsten | 0.6 | 1400 | 40 | 50 | 24 |
| Comparative Example 23 | Jet fountain | Blade | Tungsten | 0.6 | 1400 | 40 | 50 | 24 |
| Comparative Example 24 | Jet fountain | Blade | Tungsten | 0.6 | 1400 | 40 | 50 | 24 |
| Comparative Example 25 | Jet fountain | Blade | Tungsten | 0.6 | 1400 | 40 | 50 | 24 |
| Comparative Example 26 | Jet fountain | Blade | Tungsten | 0.6 | 1400 | 40 | 50 | 24 |
| Comparative Example 27 | Jet fountain | Blade | Tungsten | 0.6 | 1400 | 40 | 50 | 24 |

**[Table 35]**

| | Flattening treatment step | | | | Product grams per square meter | Raw material | | | Contaminant amount |
|---|---|---|---|---|---|---|---|---|---|
| | Stage number | Temperature | Surface roughness | Elastic roll hardness | | Waste paper | NBKP | LBKP | |
| | | °C | µm | Hv | g/m² | % | % | % | |
| Comparative Example 8 | 9 | 140 | 3 | 98 | 54.2 | 20 | 60 | 20 | 0.084 |
| Comparative Example 9 | 9 | 140 | 3 | 98 | 54.2 | 20 | 60 | 20 | 0.089 |
| Comparative Example 10 | 9 | 140 | 3 | 98 | 54.2 | 20 | 60 | 20 | 0.087 |
| Comparative Example 11 | 9 | 140 | 3 | 98 | 54.2 | 20 | 60 | 20 | 0.092 |
| Comparative Example 12 | 9 | 140 | 3 | 98 | 54.2 | 20 | 60 | 20 | 0.095 |
| Comparative Example 13 | 9 | 140 | 3 | 98 | 54.2 | 20 | 60 | 20 | 0.086 |
| Comparative Example 14 | 2 | 140 | 3 | 98 | 54.2 | 20 | 60 | 20 | 0.086 |
| Comparative Example 15 | 9 | 140 | 3 | 98 | 54.2 | 20 | 60 | 20 | 0.089 |
| Comparative Example 16 | 9 | 140 | 3 | 98 | 54.2 | 20 | 60 | 20 | 0.086 |
| Comparative Example 17 | 9 | 140 | 3 | 98 | 54.2 | 20 | 60 | 20 | 0.089 |
| Comparative Example 18 | 9 | 140 | 3 | 98 | 54.2 | 20 | 60 | 20 | 0.090 |
| Comparative Example 19 | 9 | 140 | 3 | 98 | 54.2 | 20 | 60 | 20 | 0.088 |
| Comparative Example 20 | 9 | 140 | 3 | 98 | 54.2 | 20 | 60 | 20 | 0.092 |
| Comparative Example 21 | 2 | 140 | 3 | 98 | 54.2 | 20 | 60 | 20 | 0.092 |
| Comparative Example 22 | 9 | 140 | 3 | 98 | 54.2 | 10 | 70 | 20 | 0.088 |
| Comparative Example 23 | 9 | 140 | 3 | 98 | 54.2 | 20 | 60 | 20 | 0.095 |
| Comparative Example 24 | 9 | 140 | 3 | 98 | 54.2 | 30 | 60 | 10 | 0.086 |
| Comparative Example 25 | 9 | 140 | 3 | 98 | 54.2 | 50 | 30 | 20 | 0.089 |
| Comparative Example 26 | 9 | 140 | 3 | 98 | 54.2 | 100 | - | - | 0.091 |
| Comparative Example 27 | 9 | 140 | 3 | 98 | 54.2 | 10 | 60 | 30 | 0.121 |

**[Table 36]**

| | Quality evaluation | | | | | | | | | | |
|---|---|---|---|---|---|---|---|---|---|---|---|
| | Texture | Paper breakage | Cockle | Specific volume | Glossiness | Glossiness unevenness | Printing unevenness | Rigidity | Yellow change | Productivity | Overall evaluation |
| Comparative Example 8 | 5.6 | × | Δ | 1.18 | 62 | 3 | 3 | 56 | 4 | 2 | × |
| Comparative Example 9 | 5.6 | × | × | 1.17 | 61 | 3 | 3 | 54 | 4 | 1 | × |
| Comparative Example 10 | 5.6 | × | × | 1.18 | 53 | 2 | 2 | 45 | 3 | 1 | × |
| Comparative Example 11 | 5.6 | × | × | 1.17 | 52 | 1 | 2 | 43 | 5 | 1 | × |
| Comparative Example 12 | 5.6 | × | × | 1.15 | 56 | 2 | 2 | 42 | 5 | 1 | × |
| Comparative Example 13 | 5.6 | × | × | 1.14 | 57 | 2 | 3 | 41 | 5 | 1 | × |
| Comparative Example 14 | 5.6 | ○ | ○ | 1.14 | 49 | 2 | 3 | 51 | 5 | 2 | × |
| Comparative Example 15 | 5.6 | ○ | Δ | 1.19 | 56 | 2 | 2 | 55 | 5 | 2 | × |
| Comparative Example 16 | 5.6 | ○ | Δ | 1.18 | 54 | 2 | 2 | 54 | 5 | 2 | × |
| Comparative Example 17 | 5.6 | ○ | Δ | 1.17 | 57 | 3 | 3 | 43 | 5 | 2 | × |
| Comparative Example 18 | 5.6 | ○ | Δ | 1.18 | 55 | 2 | 2 | 44 | 5 | 1 | × |
| Comparative Example 19 | 5.6 | ○ | Δ | 1.19 | 58 | 2 | 3 | 54 | 5 | 2 | × |
| Comparative Example 20 | 5.6 | ○ | Δ | 1.17 | 59 | 2 | 3 | 53 | 5 | 2 | × |
| Comparative Example 21 | 5.6 | ○ | Δ | 1.17 | 50 | 1 | 2 | 53 | 5 | 2 | × |
| Comparative Example 22 | 5.6 | × | Δ | 1.17 | 62 | 5 | 4 | 54 | 5 | 4 | × |
| Comparative Example 23 | 5.6 | × | Δ | 1.14 | 62 | 5 | 4 | 74 | 5 | 4 | × |
| Comparative Example 24 | 5.6 | × | Δ | 1.01 | 62 | 5 | 4 | 58 | 5 | 4 | × |
| Comparative Example 25 | 5.6 | × | Δ | 0.94 | 61 | 4 | 4 | 57 | 5 | 4 | × |
| Comparative Example 26 | 5.6 | × | Δ | 0.93 | 60 | 4 | 4 | 57 | 4 | 4 | × |
| Comparative Example 27 | 5.6 | × | Δ | 1.11 | 60 | 4 | 4 | 56 | 4 | 1 | × |

### "Discussions"

Examples according to the present invention shows that high quality paper can be obtained albeit in high speed paper making, as compared with the cases in Comparative Examples.

### Brief Description of the Drawings

FIG. 1 is a schematic explanatory diagram showing a first zone of an apparatus constitution example of a paper making machine.
FIG. 2 is a schematic explanatory diagram showing a second zone of an apparatus constitution example of a paper making machine.
FIG. 3 is a schematic explanatory diagram showing a third zone of an apparatus constitution example of a paper making machine.
FIG. 4 is a schematic explanatory diagram showing a forth zone of an apparatus constitution example of a paper making machine.
FIG. 5 is a schematic explanatory diagram showing a modified example of the calender part in the forth zone of an apparatus constitution example of a paper making machine.
FIG. 6 is a schematic explanatory diagram showing the ejection of paper stock of a head box.
FIG. 7 is a schematic explanatory diagram showing a heating metal roll.
FIG. 8 is a schematic explanatory diagram showing an example of an internal heating device by electromagnetic induction action.
FIG. 9 is a schematic explanatory diagram showing an example of a cleaning apparatus.
FIG. 9 is a schematic explanatory diagram showing an example of a blade coating machine.

### Description of the Symbols

1: First wire, 2: Second wire, 3: Head box, 5: Blade, 10: Twin wire former, 21: First press, 22: Presses 22, 40: Size press, 41: Air turn bar, 50: Pre-calender, 51: Metal roll, 52: Elastic roll, 60: Roll coater, 65A: First blade coater, 70: On-machine calender, M: Metal roll, D: Elastic roll, 80: Reel, 90: Applicator, 91: Blade.

## Claims

1. (Currently Amended) A process for producing a coated paper incorporating successively a step of making a paper to form a paper layer, a step of pressing the paper layer by dewatering means to form a wet paper, a step for drying the wet paper to form a dry web and a step for coating within on-machine, **characterized in**:
the step of making the paper is adapted to form the paper layer with a twin wire former in which a paper material is injected from a head box between two wires each of which loops;
the step for coating includes an undercoating step and a face coating step;
the undercoating step is adapted to apply a sizing agent as an undercoating liquid to the dry web by a size press;
a step for drying the undercoating liquid and a first flattening treatment step of performing a flattening treatment by a pre-calendar are included in this order; and
the face coating step is adapted to coat a paper to be coated, after performing the first flattening treatment step, by using an arrangement including both apparatus (1) and apparatus (2) as follows, by selecting either one apparatus from the apparatus (1) and the apparatus (2) and by coating with the selected apparatus or by performing a coating step using apparatus (2) after performing a coating step using apparatus (1)
(1) an apparatus for roll-coating, by which one side and the other side of the paper to be coated is roll-coated with an aqueous coating liquid consisting mainly of an adhesive and a pigment, an then the coated paper is dried,
(2) an apparatus for blade-coating, by which one side and the other side of the paper to be coated is blade-coated with an aqueous coating liquid consisting mainly of an adhesive and a pigment, and then the coated paper is dried.

2. (Currently Amended) The process for producing a coated paper according to claim 1, wherein the pre-calendar comprises a heated metal roll as at least one roll of a pair of rolls.

3. (Currently Amended) The process for producing a coated paper according to claims 1 or 2, wherein the pre-calendar comprises a pair of a metal roll and an elastic roll and the metal roll is heated to a temperature of 100 to 300°C.

4. (Currently Amended) An arrangement for producing a coated paper incorporating successively an apparatus for making a paper to form a paper layer, an apparatus for pressing the paper layer by dewatering means to form a wet paper, an apparatus for drying the wet paper to form a dry web and an apparatus for coating within on-machine, **characterized in**:
the apparatus for making the paper is adapted to form the paper layer with a twin wire former in which a paper material is injected from a head box between two wires each of which loops;
the apparatus for coating includes an apparatus for undercoating and an apparatus for face coating;
the apparatus for undercoating is adapted to apply a sizing agent as an undercoating liquid to the dry web by a size press
an apparatus for drying the undercoating liquid and a first flattening treatment apparatus for performing a flattening treatment by a pre-calendar are included in this order and
the apparatus for face coating is provided with both apparatus (1) and apparatus (2) as follows and is adapted to coat a paper to be coated, after performing the first flattening treatment apparatus, by selecting either one apparatus from the apparatus (1) and the apparatus (2) and by coating with the selected apparatus or by selecting apparatus (2) after selecting apparatus (1) and by coating with the selected apparatus (1,2) in this order
(1) an apparatus for roll-coating, by which one side and the other side of the paper to be coated is roll-coated with an aqueous coating liquid consisting mainly of an adhesive and a pigment, and then the coated paper is dried,
(2) an apparatus for blade-coating, by which one side and the other side of the paper to be coated is blade-coated with an aqueous coating liquid consisting mainly of an adhesive and a pigment, and then the coated paper is dried.

## Patentansprüche

1. (Aktuell geändert) Verfahren zum Herstellen eines beschichteten Papiers, das nacheinander einen Schritt zum Herstellen des Papiers, um eine Papierschicht zu bilden, einen Schritt zum Pressen der Papierschicht mit Hilfe eines Entwässerungsmittels, um ein feuchtes Papier zu bilden, einen Schritt zum Trocknen des feuchten Papiers, um eine trockene Papierbahn zu bilden, und einen Schritt zum Beschichten innerhalb einer On-Maschine umfasst, **dadurch gekennzeichnet dass**:
der Schritt zum Herstellen des Papiers dazu ausgelegt ist, die Papierschicht mit einem Doppelsiebformer zu bilden, in dem ein Papiergrundstoff aus einem Oberkasten zwischen zwei Siebe gespritzt wird, wovon jedes eine Schleife bildet;
der Schritt zum Beschichten einen Schritt zum Grundieren und einen Schritt für die Oberflächenbeschichtung umfasst;
der Schritt zum Grundieren dazu ausgelegt ist, ein Leimungsmittel als Grundierungsflüssigkeit auf die trockene Papierbahn durch eine Leimpresse aufzubringen;
ein Schritt zum Trocknen der Grundierungsflüssigkeit und ein erster Schritt eines Verfahrens zur Glättung, bei dem ein Glättungsverfahren durch einen Vor-Kalander ausgeführt wird, in diese Reihenfolge enthalten sind; und
der Schritt für die Oberflächenbeschichtung dazu ausgelegt ist, ein zu beschichtendes Papier zu beschichten, nachdem der erste Schritt des Verfahrens zur Glättung ausgeführt wurde, wobei eine Anordnung wie folgt verwendet wird, die sowohl Vorrichtung (1) als auch Vorrichtung (2) umfasst, indem eine der Vorrichtungen aus Vorrichtung (1) und Vorrichtung (2) ausgewählt wird und das Beschichten mit der ausgewählten Vorrichtung ausgeführt wird, oder durch Ausführen eines Beschichtungsschritts mit Hilfe von Vorrichtung (2), nachdem ein Beschichtungsschritt mit Hilfe von Vorrichtung (1) ausgeführt wurde:
(1) eine Vorrichtung für Walzenbeschichtung, durch die eine Seite und die andere Seite des zu beschichtenden Papiers mit einer wässrigen Beschichtungsflüssigkeit walzenbeschichtet wird, die hauptsächlich aus einem Klebemittel und einem Pigment besteht, und dann das beschichtete Papier getrocknet wird,
(2) eine Vorrichtung für Blattbeschichtung, durch die eine Seite und die andere Seite des zu beschichtenden Papiers mit einer wässrigen Beschichtungsflüssigkeit blattbeschichtet wird, die hauptsächlich aus einem Klebemittel und einem Pigment besteht, und dann das beschichtete Papier getrocknet wird.

2. (Aktuell geändert) Verfahren zum Herstellen eines beschichteten Papiers nach Anspruch 1, wobei der Vor-Kalander eine beheizte Metallwalze als mindestens eine Walze eines Walzenpaares umfasst.

3. (Aktuell geändert) Verfahren zum Herstellen eines beschichteten Papiers nach einem der Ansprüche 1 oder 2, wobei der Vor-Kalander ein Paar aus einer Metallwalze und einer elastischen Walze umfasst und die Metallwalze auf eine Temperatur von 100 bis 300 °C aufgeheizt wird.

4. (Aktuell geändert) Anordnung zum Herstellen eines beschichteten Papiers, das nacheinander eine Vorrichtung zum Herstellen eines Papiers, um eine Papierschicht zu bilden, eine Vorrichtung zum Pressen der Papierschicht mit Hilfe eines Entwässerungsmittels, um ein feuchtes Papier zu bilden, eine Vorrichtung zum Trocknen des feuchten Papiers, um eine trockene Papierbahn zu bilden, und eine Vorrichtung zum Beschichten innerhalb einer On-Maschine einschließt, **dadurch gekennzeichnet dass**:
die Vorrichtung zum Herstellen des Papiers dazu ausgelegt ist, die Papierschicht mit einem Doppelsiebformer zu bilden, in dem ein Papiergrundstoff aus einem Oberkasten zwischen zwei Siebe gespritzt wird, wovon jedes eine Schleife bildet;
die Vorrichtung zum Beschichten eine Vorrichtung zum Grundieren und eine Vorrichtung zur Oberflächenbeschichtung umfasst;
die Vorrichtung zum Grundieren dazu ausgelegt ist, ein Leimungsmittel auf die trockene Papierbahn mit Hilfe einer Leimpresse aufzubringen
eine Vorrichtung zum Trocknen der Grundierungsflüssigkeit und eine Vorrichtung für den ersten Schritt eines Verfahrens zur Glättung zum Ausführen einer Glättung durch einen Vor-Kalander, in dieser Reihenfolge enthalten sind und
die Vorrichtung für die Oberflächenbeschichtung wie folgt sowohl mit Vorrichtung (1) als auch Vorrichtung (2) ausgerüstet ist und dazu ausgelegt ist, ein zu beschichtendes Papier zu beschichten, nachdem die Vorrichtung für die erste Glättung ausgeführt wurde, indem entweder eine Vorrichtung aus der Vorrichtung (1) und der Vorrichtung (2) ausgewählt wird und das Beschichten mit der ausgewählten Vorrichtung ausgeführt wird, oder indem die Vorrichtung (2) ausgewählt wird, nachdem die Vorrichtung (1) ausgewählt wurde, und das Beschichten mit der ausgewählten Vorrichtung (1, 2) in dieser Reihenfolge ausgeführt wird:
(1) eine Vorrichtung für Walzenbeschichtung, durch die eine Seite und die andere Seite des zu beschichtenden Papiers mit einer wässrigen Beschichtungsflüssigkeit walzenbeschichtet wird, die hauptsächlich aus einem Klebemittel und einem Pigment besteht, und dann das beschichtete Papier getrocknet wird,
(2) eine Vorrichtung für Blattbeschichtung, durch die eine Seite und die andere Seite des zu beschichtenden Papiers mit einer wässrigen Beschichtungsflüssigkeit blattbeschichtet wird, die hauptsächlich aus einem Klebemittel und einem Pigment besteht, und dann das beschichtete Papier getrocknet wird.

## Revendications

1. Procédé de fabrication de papier couché mettant successivement en oeuvre une étape de fabrication de papier pour former une couche de papier, une étape de pressage de la couche de papier par un moyen de déshydratation pour former du papier humide, une étape de séchage du papier humide pour former une bobine sèche et une étape de couchage sur machine, **caractérisé en ce que** :
l'étape de fabrication du papier est adaptée pour former la couche de papier avec un formeur à double toile où un matériau de papier est injecté à partir d'une caisse de tête entre deux toiles dont chacune fait une boucle ;
l'étape de couchage comporte une étape de sous-couchage et une étape de couchage en surface ;
l'étape de sous-couchage est adaptée pour appliquer un agent d'encollage sous forme de liquide de sous-couchage à la bobine sèche par une presse encolleuse ;
une étape de séchage du liquide de sous-couchage et une première étape de traitement d'aplatissement pour réaliser un traitement d'aplatissement par un pré-calendrier sont inclus dans cet ordre ; et
l'étape de couchage en surface est adaptée pour coucher du papier devant être couché, après réalisation de la première étape de traitement d'aplatissement, en utilisant un agencement comportant un appareil (1) et un appareil (2) comme suit, soit en sélectionnant un appareil parmi l'appareil (1) et l'appareil (2) et en couchant avec l'appareil sélectionné ou en réalisant une étape de couchage en utilisant l'appareil (2) après la réalisation d'une étape de couchage en utilisant l'appareil (1) ;
(1) un appareil pour un couchage par rouleau, moyennant quoi une face et l'autre face du papier à coucher est couchée au rouleau avec un liquide de couchage aqueux essentiellement constitué d'un adhésif et d'un pigment, et ensuite le papier couché est séché,
(2) un appareil pour un couchage à la lame, moyennant quoi une face et l'autre face du papier à coucher est couchée à la lame avec un liquide de couchage aqueux essentiellement constitué d'un adhésif et d'un pigment, et ensuite le papier couché est séché.

2. Procédé de fabrication de papier couché selon la revendication 1, dans lequel le pré-calendrier comprend un rouleau métallique chauffé tel qu'au moins un rouleau d'une paire de rouleaux.

3. Procédé de fabrication de papier couché selon la revendication 1 ou 2, dans lequel le pré-calendrier comprend une paire d'un rouleau métallique et d'un rouleau danseur et le rouleau métallique est chauffé à une température de 100 à 300°C.

4. Agencement de fabrication de papier couché mettant successivement en oeuvre un appareil pour fabriquer du papier afin de former une couche de papier, un appareil pour presser la couche de papier par un moyen de déshydratation afin de former du papier humide, un appareil pour sécher le papier humide afin de former une bobine sèche et un appareil de couchage sur machine, **caractérisé en ce que** :
l'appareil de fabrication de papier est adapté pour former la couche de papier avec un formeur à double toile où un matériau de papier est injecté à partir d'une caisse de tête entre deux toiles dont chacune fait une boucle ;
l'appareil de couchage comporte un appareil pour le sous-couchage et un appareil pour le couchage en surface ;
l'appareil de sous-couchage est adapté pour appliquer un agent d'encollage sous forme de liquide de sous-couchage à la bobine sèche par une presse encolleuse
un appareil de séchage du liquide de sous-couchage et un premier appareil de traitement d'aplatissement permettant de réaliser un traitement d'aplatissement par un pré-calendrier sont inclus dans cet ordre ; et
l'appareil de couchage en surface est pourvu d'un appareil (1) et d'un appareil (2) comme suit et est adapté pour coucher du papier devant être couché, après mise en oeuvre du premier appareil de traitement d'aplatissement, soit en sélectionnant un appareil de l'appareil (1) et de l'appareil (2) et en couchant à l'aide de l'appareil sélectionné ou en sélectionnant l'appareil (2) après la sélection de l'appareil (1) et en couchant à l'aide de l'appareil sélectionné (1, 2) dans cet ordre
(1) un appareil de couchage par rouleau, moyennant quoi une face et l'autre face du papier à coucher sont couchées au rouleau avec un liquide de couchage aqueux essentiellement constitué d'un adhésif et d'un pigment, et ensuite le papier couché est séché,
(2) un appareil de couchage à la lame, moyennant quoi une face et l'autre face du papier à coucher sont couchées à la lame avec un liquide de couchage aqueux essentiellement constitué d'un adhésif et d'un pigment, et ensuite le papier couché est séché.
